



US008809415B2

(12) **United States Patent**  
**Petricchio et al.**

(10) **Patent No.:** **US 8,809,415 B2**  
(45) **Date of Patent:** **\*Aug. 19, 2014**

(54) **GOLF BALL HAVING A COVER LAYER  
WITH A PURPOSED HARDNESS GRADIENT**

(75) Inventors: **Randy Petrichko**, Fairhaven, MA (US); **Shawn Ricci**, Fairhaven, MA (US); **Edmund A. Hebert**, Fairhaven, MA (US); **Brian Comeau**, Fairhaven, MA (US); **David A. Bulpett**, Fairhaven, MA (US)

(73) Assignee: **Acushnet Company**, Fairhaven, MA (US)

(\*) Notice: Subject to any disclaimer, the term of this patent is extended or adjusted under 35 U.S.C. 154(b) by 985 days.

This patent is subject to a terminal disclaimer.

(21) Appl. No.: **12/187,046**

(22) Filed: **Aug. 6, 2008**

(65) **Prior Publication Data**

US 2009/0286629 A1 Nov. 19, 2009

**Related U.S. Application Data**

(63) Continuation-in-part of application No. 12/122,396, filed on May 16, 2008.

(51) **Int. Cl.**

**A63B 37/12** (2006.01)  
**A63B 37/00** (2006.01)  
**C08G 18/62** (2006.01)  
**C08G 18/86** (2006.01)

(52) **U.S. Cl.**

USPC ..... **522/174**; 525/131; 528/60; 528/68; 528/75; 473/378

(58) **Field of Classification Search**

None

See application file for complete search history.

(56) **References Cited**

**U.S. PATENT DOCUMENTS**

|             |         |                    |       |           |
|-------------|---------|--------------------|-------|-----------|
| 3,652,520 A | 3/1972  | Ryan et al.        | ..... | 260/86.1  |
| 4,560,168 A | 12/1985 | Aoyama             | ..... | 273/232   |
| 4,658,062 A | 4/1987  | Hinney et al.      | ..... | 564/305   |
| 4,960,281 A | 10/1990 | Aoyama             | ..... | 273/232   |
| 4,994,621 A | 2/1991  | Yeakey et al.      | ..... | 564/475   |
| 5,334,673 A | 8/1994  | Wu                 | ..... | 273/235 R |
| 5,484,870 A | 1/1996  | Wu                 | ..... | 528/28    |
| 5,688,191 A | 11/1997 | Cavallaro et al.   | ..... | 473/373   |
| 5,692,974 A | 12/1997 | Wu et al.          | ..... | 473/377   |
| 5,713,801 A | 2/1998  | Aoyama             | ..... | 473/354   |
| 5,803,831 A | 9/1998  | Sullivan et al.    | ..... | 473/374   |
| 5,849,168 A | 12/1998 | Lutz               | ..... | 264/755   |
| 5,885,172 A | 3/1999  | Hebert et al.      | ..... | 473/354   |
| 5,908,358 A | 6/1999  | Wu                 | ..... | 473/378   |
| 5,919,100 A | 7/1999  | Boehm et al.       | ..... | 473/354   |
| 5,965,669 A | 10/1999 | Cavallaro et al.   | ..... | 525/221   |
| 5,981,654 A | 11/1999 | Rajagopalan        | ..... | 525/66    |
| 5,981,658 A | 11/1999 | Rajagopalan et al. | ..... | 525/72    |
| 6,056,842 A | 5/2000  | Dalton et al.      | ..... | 156/243   |
| 6,149,535 A | 11/2000 | Bissonnette et al. | ..... | 473/354   |

|                   |         |                    |       |            |
|-------------------|---------|--------------------|-------|------------|
| 6,180,040 B1      | 1/2001  | Ladd et al.        | ..... | 264/248    |
| 6,180,722 B1      | 1/2001  | Dalton et al.      | ..... | 525/193    |
| 6,207,784 B1      | 3/2001  | Rajagopalan        | ..... | 528/71     |
| 6,386,992 B1      | 5/2002  | Harris et al.      | ..... | 473/371    |
| 6,503,156 B1      | 1/2003  | Sullivan           | ..... | 473/374    |
| 6,506,130 B2      | 1/2003  | Sullivan           | ..... | 473/374    |
| 6,831,136 B2      | 12/2004 | Chao et al.        | ..... | 525/377    |
| 6,835,794 B2      | 12/2004 | Wu et al.          | ..... | 528/64     |
| 7,211,624 B2      | 5/2007  | Wu et al.          | ..... | 525/92 C   |
| 7,427,242 B1 *    | 9/2008  | Sullivan et al.    | ..... | 473/373    |
| 7,481,956 B2      | 1/2009  | Wu et al.          | ..... | 264/255    |
| 7,964,668 B2 *    | 6/2011  | Petricchio et al.  | ..... | 525/131    |
| 8,039,573 B2 *    | 10/2011 | Petricchio et al.  | ..... | 528/60     |
| 8,246,884 B2 *    | 8/2012  | Petricchio et al.  | ..... | 264/279.1  |
| 2001/0009310 A1   | 7/2001  | Hebert             | ..... |            |
| 2001/0018375 A1   | 8/2001  | Hayashi            | ..... |            |
| 2001/0019971 A1   | 9/2001  | Hayashi            | ..... |            |
| 2002/0025862 A1   | 2/2002  | Sullivan           | ..... |            |
| 2002/0028885 A1   | 3/2002  | Sullivan           | ..... |            |
| 2002/0167116 A1 * | 11/2002 | Inoue et al.       | ..... | 264/331.11 |
| 2003/0199337 A1   | 10/2003 | Hebert             | ..... |            |
| 2003/0212240 A1   | 11/2003 | Wu                 | ..... |            |
| 2004/0019138 A1 * | 1/2004  | Voorheis et al.    | ..... | 524/100    |
| 2004/0053709 A1   | 3/2004  | Sullivan           | ..... |            |
| 2004/0097653 A1 * | 5/2004  | Kim et al.         | ..... | 525/130    |
| 2004/0217516 A1   | 11/2004 | Moriyama           | ..... |            |
| 2004/0220356 A1   | 11/2004 | Wu                 | ..... |            |
| 2004/0259665 A1 * | 12/2004 | Sullivan et al.    | ..... | 473/371    |
| 2005/0079351 A1   | 4/2005  | Isogawa            | ..... |            |
| 2005/0176524 A1   | 8/2005  | Sullivan           | ..... |            |
| 2006/0009309 A1 * | 1/2006  | Rajagopalan et al. | ..... | 473/371    |
| 2006/0017201 A1   | 1/2006  | Wu                 | ..... |            |
| 2006/0116481 A1   | 6/2006  | Morgan             | ..... |            |
| 2007/0270242 A1 * | 11/2007 | Keller et al.      | ..... | 473/371    |
| 2009/0286624 A1 * | 11/2009 | Petricchio et al.  | ..... | 473/377    |
| 2009/0286627 A1 * | 11/2009 | Petricchio et al.  | ..... | 473/378    |

**OTHER PUBLICATIONS**

Huang, Gas Permeability of Crosslinked HTPB-H12MDI-Based Polyurethane Membrane, Journal of Applied Polymer Science vol. 58, 1995 p. 1913-1923.\*  
Technical Information for Di-Cup; Arkema Inc; pp. 1-4 no date.\*  
Non-Final Office Action dated Aug. 25, 2009 of corresponding U.S. Appl. No. 12/122,396.  
Non-Final Office Action dated Nov. 10, 2009 of corresponding U.S. Appl. No. 12/122,396.  
Final Office Action dated May 24, 2010 of corresponding U.S. Appl. No. 12/122,396.  
Final Office Action dated Feb. 16, 2011 of corresponding U.S. Appl. No. 12/122,396.  
Non-Final Office Action dated Sep. 1, 2010 of corresponding U.S. Appl. No. 12/122,396.  
Final Office Action dated Feb. 16, 2011 issued in U.S. Appl. No. 12/122,396.

\* cited by examiner

*Primary Examiner* — David Buttner

(74) *Attorney, Agent, or Firm* — Smith, Gambrell & Russell, LLP

(57) **ABSTRACT**

Compositions for golf balls that include polyurethane and/or polyurea linkages and that are crosslinked in the soft segments of the polymer backbone to improve the crosslink density and effect a hardness gradient throughout the molded article.



***FIG. 1***



***FIG. 2***



**FIG. 3**



**FIG. 4**



FIG. 5a



FIG. 5b

## 1

**GOLF BALL HAVING A COVER LAYER  
WITH A PURPOSED HARDNESS GRADIENT**CROSS-REFERENCE TO RELATED  
APPLICATIONS

This application is a continuation-in-part of U.S. patent application Ser. No. 12/122,396, filed May 16, 2008, now pending, the entire disclosure of which is incorporated by reference herein.

## FIELD OF THE INVENTION

The present invention relates to golf balls that have a cover layer with a purposed hardness gradient. In particular, the compositions of the invention, which include a polymer backbone including hydrocarbons and urea linkages, urethane linkages, or a combination of both types of linkages, are crosslinked both in the soft and hard segments to provide a material with higher hardness than conventional polyurethane and polyurea compositions. The compositions of the invention may be used in any outer layer of a golf ball, e.g., an outer cover layer or inner cover layer, or may be used as a coating to be disposed over a structural outer layer of a golf ball.

## BACKGROUND OF THE INVENTION

Golf ball manufacturers have been experimenting with various materials and manufacturing methods for golf balls over the years in an attempt to improve overall performance and durability and to further refine the manufacturing process.

For example, over the past years, golf ball manufacturers have been using ionomer resins for golf ball cover materials because of the durability, rebound, and scuff resistance characteristics of the materials. However, while ionomer resins are more durable than other types of golf ball layer materials, the same properties that result in durability also provide a hard "feel" and generally result in a lower spin rate and, thus, lower control, due to the hardness of the material.

Alternatively, polyurethane compositions produce "soft" covers and typically allow for greater control because of the increased spin. Because conventional polyurethane cover materials are typically formed of aromatic components, the ultraviolet degradation of the material, which leads to yellowing, led to the recent trend toward light stable cover materials, such as aliphatic polyurethane and polyurea materials. Whether aromatic or aliphatic in nature, however, the relative softness of the polyurethane and polyurea materials introduces durability issues.

Further attempts to compensate for the "hard" feel of ionomer-covered golf balls and durability and adhesion issues with polyurethane-covered and polyurea-covered golf balls have resulted in blends of hard ionomer resins, i.e., resins with hardness values of about 60 Shore D and above, with relatively softer polymeric materials. For example, blends of hard ionomers with polyurethanes have been used to form intermediate layers and cover layers of golf balls. However, such blends generally have processing difficulties associated with their use in the production of golf balls due to the incompatibility of the components. In addition, golf balls produced from these incompatible mixtures will have inferior golf ball properties such as poor durability, cut resistance, and the like.

As such, a need exists in the golf ball art for materials that have the performance benefits of polyurethane and polyurea, but higher hardness and higher flexural modulus values, as

## 2

well as improved hydrophobicity. In addition, golf balls having layers formed, at least in part, from such compositions would be advantageous. The present invention addresses such materials, methods of forming the materials, and portions of golf balls formed from these materials.

## SUMMARY OF THE INVENTION

The present invention relates to a golf ball including a core and a cover, wherein the cover includes a single layer formed from the reaction product of a conjugated diene including a plurality of terminal ends including amino groups, hydroxy groups, or a combination thereof; an isocyanate-containing component; and a curative blend including an amine-terminated curing agent, a hydroxy-terminated curing agent, or a combination thereof, and an organic peroxide; wherein the cover has a first hardness at an interior location on the layer at least about 10 percent less than a second hardness at an exterior location on the layer.

In one embodiment, the conjugated diene includes a polybutadiene including a plurality terminal ends including amino groups, hydroxy groups, or a combination thereof. In another embodiment, the plurality of terminal ends include primary amino groups, secondary amino groups, or a combination thereof. In yet another embodiment, the plurality of terminal ends include primary hydroxy groups, secondary hydroxy groups, or a combination thereof.

In this aspect of the invention, the first hardness is at least about 12 percent less than the second hardness. In one embodiment, the first hardness is about 20 percent to about 35 percent less than the second hardness.

The curative blend may further include a photoinitiator.

The present invention is also directed to a method of forming a golf ball including the steps of:

providing a core;  
forming a prepolymer including the reaction product of an isocyanate-containing component and a first isocyanate-reactive component, wherein the first isocyanate-reactive component includes a conjugated diene hydrocarbon including at least two functional groups including amino groups, hydroxy groups, or a mixture thereof, and wherein the prepolymer includes about 5 weight percent to about 9 weight percent NCO groups;

mixing the prepolymer with a curative blend including a second isocyanate-reactive component and at least one free radical initiator to form a mixture;  
placing a first portion of the mixture in a first cavity of a first mold half for a predetermined gel time at a first mold temperature;

positioning the core within the first cavity;  
placing a second portion of the mixture in a second cavity of a second mold half for the predetermined gel time at the first mold temperature;

mating the first and second mold halves; and  
raising the first mold temperature to a second mold temperature for a predetermined period of time to form a cured cover having a hardness gradient from an interior location on the cover to an exterior location on the cover of about 5 percent or greater.

In one embodiment, the hardness gradient is about 10 percent or greater. In another embodiment, the hardness gradient is about 20 percent to about 35 percent. In yet another embodiment, the at least one free radical initiator includes peroxide. In still another embodiment, the first isocyanate-reactive component includes hydroxy-terminated polybutadiene. In another embodiment, the first isocyanate-reactive component includes amine-terminated polybutadiene. In yet

another embodiment, the second isocyanate-reactive component includes terminal amino groups, terminal hydroxy groups, or a combination thereof.

The present invention also relates a method of forming a golf ball including a core and a cover including the steps of:

- providing a core;
- providing a conjugated diene including a plurality of terminal ends including amino groups, hydroxy groups, or a combination thereof;
- providing an isocyanate-containing component;
- reacting the conjugated diene with the isocyanate-containing component to form a prepolymer;
- forming a curative blend including:
- an amine-terminated component, a hydroxy-terminated component, or a combination thereof; and
- a free radical initiator;
- reacting the prepolymer and curative blend to form a composition including crosslinks between the hydrocarbons; and
- casting a cover about the core from the composition, wherein the cover has a hardness gradient that increases from an interior location to an exterior location of at least about 10 percent.

In one embodiment, the free radical initiator includes an organic peroxide. In another embodiment, the step of casting includes the steps of:

- placing a first portion of the composition in a first cavity of a first mold half for a predetermined gel time at a first mold temperature;
- positioning the core within the first cavity;
- placing a second portion of the composition in a second cavity of a second mold half for the predetermined gel time at the first mold temperature;
- mating the first and second mold halves; and
- raising the first mold temperature to a second mold temperature for a predetermined period of time to form a cured cover.

In another embodiment, the hardness gradient is about 15 percent or greater. In yet another embodiment, the predetermined period of time is about 2 minutes to about 12 minutes. In still another embodiment, the curative blend further includes a photoinitiator.

#### BRIEF DESCRIPTION OF THE DRAWINGS

Further features and advantages of the invention can be ascertained from the following detailed description that is provided in connection with the drawing(s) described below:

FIG. 1 is a cross-sectional view of a two-piece golf ball, wherein the cover is formed from a composition of the invention;

FIG. 2 is a cross-sectional view of a multi-component golf ball, wherein at least one layer is formed from a composition of the invention;

FIG. 3 is a cross-sectional view of a multi-component golf ball having a large core, wherein at least one layer is formed from a composition of the invention;

FIG. 4 is a cross-sectional view of a multi-component golf ball including a dual core and a dual cover, wherein at least one layer is formed from a composition of the invention;

FIG. 5a is a cross-sectional view of a golf ball with a cover having a purposed hardness gradient according to the invention; and

FIG. 5b is an illustration of the hardness gradient in a button formed from the compositions of the invention.

#### DETAILED DESCRIPTION OF THE INVENTION

Because crosslinking in conventional castable reactive liquid materials is limited to the hard segments, i.e., the isocyanate groups, the ability to increase crosslinking density and, thus, hardness is limited. Thus, the present invention relates to compositions for use in golf balls that include polyurethane systems, polyurea systems, and mixtures thereof that are crosslinked both in the hard and soft segments of the polymer.

In particular, the compositions of the invention include the reaction product of an isocyanate-containing component and an isocyanate-reactive component that is subjected to a curing process that involves a first curative that crosslinks the hard segments in the polymer and a second curative that crosslinks the soft segments to produce a layer that has a purposed hardness gradient.

The compositions of the invention provide an alternative to thermoplastic materials, such as ionomers, that are typically used as outer covers on large core balls or inner covers on multilayer balls with relatively soft covers. In fact, without being bound to any particular theory, golf balls that include the compositions of the invention as cover layers have improved moisture resistance and durability. As such, golf balls of the present invention, e.g., golf balls including single cover layers formed from the compositions of the invention, may replace conventional golf balls including a dual cover system with a hard inner cover layer and a soft outer cover layer at least because the purposed hardness gradient in the single cover layer will provide the benefits previously achieved with the dual cover system. In addition, the compositions of the invention may be used in an inner cover layer.

The present invention also explores the methods of making such compositions and other golf ball constructions that incorporate the compositions of the invention in at least a portion thereof. In fact, the compositions of the invention can be used with a variety of golf ball constructions. For example, the compositions of the invention may be used as a cover layer in a two-piece ball with a large core, an outer cover layer in a three-piece ball with a relatively thin inner cover layer, an intermediate layer in a three-piece ball, or an inner cover layer in a golf ball having dual cover layers. In addition, the compositions of the invention may be used to form coatings for golf balls. The composition components, golf ball constructions, and layer and ball properties are discussed in greater detail below.

#### THE COMPOSITIONS OF THE INVENTION

The compositions of the invention include a prepolymer that is the reaction product of an isocyanate-containing component and an isocyanate-reactive component, which is crosslinked with a combination of a curing agent and a free radical initiator. In particular, the reaction product of the isocyanate-containing component and isocyanate-reactive component produces a prepolymer including polyurethane linkages, polyurea linkages, or a combination thereof. The components of the composition are discussed below.

##### Prepolymer

The prepolymer used in the compositions of the invention may be based on a polyurethane, a polyurea, or a combination thereof. For example, the prepolymer may include urethane linkages, which is referred to herein as a polyurethane prepolymer, urea linkages, which is referred to herein as a polyurea prepolymer, or urethane and urea linkages, which is referred to herein as a hybrid prepolymer, each of which are discussed in more detail below.

##### Polyurethane Prepolymer

When based on polyurethane, the prepolymer is a product formed by a reaction between at least one isocyanate and at least one hydroxy-terminated component. The components of the polyurethane prepolymer may be aromatic, aromatic-

aliphatic, or aliphatic, which provide varying degrees of light stability. As used herein, aromatic aliphatic compounds should be understood as those containing an aromatic ring, wherein the isocyanate group is not directly bonded to the ring.

Along a continuum, an aromatic composition is less light stable than an aromatic-aliphatic composition, which is less light stable than an aliphatic composition. For example, an aliphatic composition made according to the invention includes only saturated components, i.e., components substantially free of unsaturated carbon-carbon bonds or aromatic groups, the use of which prevents yellowing over time. The term "saturated," as used herein, refers to compositions having saturated aliphatic and alicyclic polymer backbones, i.e., with no carbon-carbon double bonds. It is important to note, however, that aromatic compositions made according to the invention may include light stabilizers to improve light stability. Thus, light stability may be accomplished in a variety of ways for the purposes of this application.

Isocyanates for use with the polyurethane prepolymer include aliphatic, cycloaliphatic, aromatic aliphatic, aromatic, derivatives thereof, and combinations of these compounds having two or more isocyanate (NCO) groups per molecule. As briefly mentioned above, however, the isocyanate may be saturated to improve the light stability of the composition of the invention. The isocyanates may be organic polyisocyanate-terminated precursors, low free isocyanate precursors, and mixtures thereof. The isocyanate component may also include any isocyanate-functional monomer, dimer, trimer, or multimeric adduct thereof, precursor, quasi-precursor, or mixtures thereof. Isocyanate-functional compounds may include monoisocyanates or polyisocyanates that include any isocyanate functionality of two or more.

Suitable isocyanate-containing components include diisocyanates having the generic structure:  $O=C=N-R-N=C=O$ , where R is preferably a cyclic or linear or branched hydrocarbon moiety containing from about 1 to 20 carbon atoms. The diisocyanate may also contain one or more cyclic groups. When multiple cyclic groups are present, linear and/or branched hydrocarbons containing from about 1 to 10 carbon atoms can be present as spacers between the cyclic groups. In some cases, the cyclic group(s) may be substituted at the 2-, 3-, and/or 4-positions, respectively. Substituted groups may include, but are not limited to, halogens, primary, secondary, or tertiary hydrocarbon groups, or a mixture thereof.

Examples of saturated (aliphatic) diisocyanates that can be used in the polyurethane precursor include, but are not limited to, ethylene diisocyanate; propylene-1,2-diisocyanate; tetramethylene diisocyanate; tetramethylene-1,4-diisocyanate; 1,6-hexamethylene diisocyanate (HDI); HDI biuret prepared from HDI; octamethylene diisocyanate; decamethylene diisocyanate; 2,2,4-trimethylhexamethylene diisocyanate; 2,4,4-trimethylhexamethylene diisocyanate; dodecane-1,2-diisocyanate; cyclobutane-1,3-diisocyanate; cyclohexane-1,2-diisocyanate; cyclohexane-1,3-diisocyanate; cyclohexane-1,4-diisocyanate; methylcyclohexylene diisocyanate (HTDI); 2,4-methylcyclohexane diisocyanate; 2,6-methylcyclohexane diisocyanate; 4,4'-dicyclohexyl diisocyanate; 2,4'-dicyclohexyl diisocyanate; 1,3,5-cyclohexane trisocyanate; isocyanatomethylcyclohexane isocyanate; 1-isocyanato-3,3,5-trimethyl-5-isocyanatomethylcyclohexane; isocyanatoethylcyclohexane isocyanate; bis(isocyanatomethyl)-cyclohexane diisocyanate; 4,4'-bis(isocyanatomethyl)dicyclohexane;

2,4'-bis(isocyanatomethyl)dicyclohexane; isophorone diisocyanate (IPDI); triisocyanate of HDI; triisocyanate of 2,2,4-trimethyl-1,6-hexane diisocyanate (TMDI); 4,4'-dicyclohexylmethane diisocyanate (H<sub>12</sub>MDI); 2,4-hexahydrotoluene diisocyanate; 2,6-hexahydrotoluene diisocyanate; aromatic aliphatic isocyanate, such as 1,2-, 1,3-, and 1,4-xylene diisocyanate; meta-tetramethylxylene diisocyanate (m-TMXDI); para-tetramethylxylene diisocyanate (p-TMXDI); trimerized isocyanurate of any polyisocyanate, such as isocyanurate of toluene diisocyanate, trimer of diphenylmethane diisocyanate, trimer of tetramethylxylene diisocyanate, isocyanurate of hexamethylene diisocyanate, isocyanurate of isophorone diisocyanate, and mixtures thereof; dimerized uretdione of any polyisocyanate, such as uretdione of toluene diisocyanate, uretdione of hexamethylene diisocyanate, and mixtures thereof; modified polyisocyanate derived from the above isocyanates and polyisocyanates; and mixtures thereof. In one embodiment, the saturated diisocyanates include isophoronediisocyanate (IPDI), 4,4'-dicyclohexylmethane diisocyanate (H<sub>12</sub>MDI), 1,6-hexamethylene diisocyanate (HDI), or a combination thereof.

As briefly discussed, aromatic aliphatic isocyanates may also be used to form the polyurethane precursor. While use of aromatic aliphatic materials does not confer the same amount of light stability to the resultant product compared to those including purely aliphatic materials, it does provide a greater degree of light stability to the resultant product compared to those formed with purely aromatic materials. Examples of aromatic aliphatic isocyanates include 1,2-, 1,3-, and 1,4-xylene diisocyanate; meta-tetramethylxylene diisocyanate (m-TMXDI); para-tetramethylxylene diisocyanate (p-TMXDI); trimerized isocyanurate of any polyisocyanate, such as isocyanurate of toluene diisocyanate, trimer of diphenylmethane diisocyanate, trimer of tetramethylxylene diisocyanate, isocyanurate of hexamethylene diisocyanate, and mixtures thereof; dimerized uretdione of any polyisocyanate, such as uretdione of toluene diisocyanate, uretdione of hexamethylene diisocyanate, and mixtures thereof; a modified polyisocyanate derived from the above isocyanates and polyisocyanates; and mixtures thereof. In addition, the aromatic aliphatic isocyanates may be mixed with any of the saturated isocyanates listed above for the purposes of this invention.

Unsaturated diisocyanates, i.e., aromatic compounds, may also be used with the present invention, although the use of unsaturated compounds in the precursor is preferably coupled with the use of a light stabilizer or pigment as discussed below. Examples of unsaturated diisocyanates include, but are not limited to, substituted and isomeric mixtures including 2,2'-, 2,4'-, and 4,4'-diphenylmethane diisocyanate (MDI), 3,3'-dimethyl-4,4'-biphenyl diisocyanate (TODI), toluene diisocyanate (TDI), polymeric MDI (PMDI, a brown liquid composed of approximately 50% methylene diisocyanate with the remainder comprised of oligomers of MDI), carbodiimide-modified liquid 4,4'-diphenylmethane diisocyanate, para-phenylene diisocyanate (PPDI), meta-phenylene diisocyanate (MPDI), triphenylmethane-4,4'-, and triphenylmethane-4,4'-trisocyanate, naphthylene-1,5-diisocyanate, 2,4'-, 4,4'-, and 2,2'-biphenyl diisocyanate, polyphenylene polymethylene polyisocyanate (PMDI) (also known as polymeric PMDI), and mixtures thereof.

An isocyanate group reacts with the hydroxy groups of the hydroxy-terminated component to form a repeating urethane linkage, which has the following general structure:



where x is the number of repeat units, i.e., about 1 or greater, and R includes straight chain or branched hydrocarbon chains having about 1 to about 20 carbons, phenyl groups, and mixtures thereof, and R<sub>1</sub> is a straight chain or branched hydrocarbon chain having about 1 to about 20 carbons.

The hydroxy-terminated component suitable for the present invention may be organic, modified organic, saturated, aliphatic, alicyclic, unsaturated, araliphatic, aromatic, substituted, or unsubstituted in nature. The hydroxy-terminated component may be hydroxy-terminated polyhydrocarbons including, but not limited to, hydroxy-terminated polybutadiene, hydroxy-terminated polyisoprene; poly(hydrogenated isoprene)polyol; poly(hydrogenated butadiene)polyol; and mixtures thereof.

In particular, the hydroxy-terminated component preferably has two or more reactive hydrogen groups per molecule, such as primary or secondary hydroxy groups, and at least one conjugated diene hydrocarbon. The conjugated diene hydrocarbon may be unsubstituted, 2-substituted, or 2,3-disubstituted 1,3-dienes or 4 up to about 12 carbon atoms. In one embodiment, the diene has up to 6 carbon atoms and the substituents in the 2- and/or 3-position may be H, alkyl, preferably lower alkyl, aryl, halogen, and mixtures thereof. The diene may be 1,3-butadiene, isoprene, 2-cyano-1,3-butadiene, 2,3-dimethyl-1,3-butadiene, 2-phenyl-1,3-butadiene, 2-methyl-3-phenyl-1,3-butadiene, and the like.

the hydroxyl functionality of the HTPB is about 2.2 to about 2.6 per chain. Because the hydroxyl functionality has an effect on the viscosity during prepolymer preparation, in one embodiment, the hydroxyl functionality of the HTPB is about 2.0 to about 2.3 per chain. In fact, the use of a HTPB with lower hydroxyl functionality may alleviate the need for more isocyanate, which increases cost and handling issues, to reduce the viscosity

10 Those of ordinary skill in the art would be aware of suitable methods to synthesize HTPB for use in the present invention. For example, diene monomers and hydrogen peroxide in a solvent are subjected to free radical addition polymerization using hydrogen peroxide as the catalyst. As recognized by a skilled artisan, the ratio of cis-1,4 and trans-1,4 and 1,2-vinyl unsaturation that occurs in the diene polymers, the number and location of hydroxyl groups, and the molecular weight of the HTPB may be a function of the polymerization temperature and the type of addition polymerization system 15 employed in forming the polymer.

20 Further examples of HTPB and methods of preparing HTPB are provided in U.S. Pat. No. 3,652,520, the disclosure of which is incorporated by reference herein. HTPB is also commercially available from Sartomer as Poly bd® resins, including Poly bd® R-45HTLO and R-20LM, and Krasol® LBH resins.

25 When a diisocyanate is reacted with a hydroxy-terminated component of the present invention, long polymer chains are formed. A general reaction scheme between a diisocyanate and a hydroxy-terminated component having primary hydroxy groups according to the invention is as follows:



In one embodiment, the hydroxy-terminated component includes hydroxy-terminated polybutadiene (HTPB) where the functional hydroxy groups are primary hydroxy groups, secondary hydroxy groups, or a combination thereof. The HTPB may have a hydroxyl functionality of about 1.8 to about 3 per chain. In one embodiment, the hydroxyl functionality is about 2 to about 3 per chain. In another embodiment,

50 where n is the number of repeat units, i.e., about 1 or greater, and R is a straight chain or branched hydrocarbon chain having about 1 to about 20 carbons, a phenyl group, or a mixture thereof.

In addition, when the hydroxy-terminated component includes secondary hydroxy groups, the reaction scheme is as follows:



-continued



where n is the number of repeat units, i.e., about 1 or greater, and R and R<sub>1</sub> are independently straight chains or branched hydrocarbon chains having about 1 to about 20 carbons, a phenyl group, or a mixture thereof.

Furthermore, when the hydroxy-terminated component includes a mixture of primary and secondary hydroxy-terminated components, the reaction scheme is as follows:

15 about 4.5 weight percent to about 10 weight percent. In still another embodiment, the NCO content ranges from about 5 weight percent to about 9 weight percent.

As known to those of ordinary skill in the art, the polyurethane prepolymer contains some amount of free isocyanate monomer. Thus, in one embodiment, the polyurethane prepolymer is stripped of free isocyanate monomer. For



where n is the number of repeat units, i.e., about 1 or greater, and R and R<sub>1</sub> are independently straight chains or branched hydrocarbon chains having about 1 to about 20 carbons, a phenyl group, or a mixture thereof.

The hydroxy-terminated component may also be blended with other hydroxyl-terminated components including, but not limited to, hydroxy-terminated polyester, hydroxy-terminated polyether, hydroxy-terminated polycarbonate, hydroxy-terminated polycaprolactones, hydroxy-terminated polyhydrocarbons, hydroxy-terminated acid functional oligomers or polymers (or ionomers thereof derived from partial or full neutralization with organic or inorganic cations)

As known to those of ordinary skill in the art, an increase in NCO content typically results in an increase in overall hardness. Thus, conventional polyurethane and polyurea compositions require an increase in NCO content to achieve high hardness values. However, increases in NCO content also lead to significant increases in reaction rates. As such, in many formulations, the fast reaction rates lead to processing issues. The compositions of the invention allow for high hardness values to be achieved with moderate NCO content and manageable reaction rates.

In one embodiment, the NCO content in the prepolymer ranges from about 4 percent to about 15 percent by weight. In another embodiment, the NCO content in the prepolymer is from about 4 to about 11 percent by weight. In yet another embodiment, the NCO content in the prepolymer ranges from

40 about 4.5 weight percent to about 10 weight percent. In still another embodiment, the NCO content ranges from about 5 weight percent to about 9 weight percent.

#### Polyurea Prepolymer

The prepolymer may also be based on a urea linkages, where the prepolymer is a product formed by a reaction between at least one isocyanate-containing component and at least one amine-terminated component. For the purposes of the present invention, the polyurea prepolymers include primarily urea linkages having the following general structure:



55 where x is the number of repeat units, i.e., about 1 or greater, and R includes straight chain or branched hydrocarbon chains having about 1 to about 20 carbons, phenyl groups, and mixtures thereof, and R<sub>1</sub> is a straight chain or branched hydrocarbon chain having about 1 to about 20 carbons.

60 Because the main difference between the polyurethane prepolymer discussed above and the polyurea prepolymer discussed in this section is the substitution of the hydroxy-

11

terminated component with an amine-terminated component, the isocyanates suitable for inclusion in the polyurea prepolymers are the same as those listed above with respect to the polyurethane prepolymers, and, thus, are incorporated by reference here. And, as above, while saturated isocyanates are preferred, aromatic aliphatic isocyanates and aromatic isocyanates are contemplated for use with the present invention.

It should be understood, however, that a prepolymer including primarily urea linkages may have distinctly different properties than a prepolymer including primarily urethane linkages due to the substitution of the hydroxy-terminated component with the amine-terminated component. For example, when a polyurea prepolymer is used, the resulting composition may have different shear, cut, resiliency, and adhesion properties than a composition with formed from a polyurethane prepolymer.

The amine-terminated component suitable for the present invention may be organic, modified organic, saturated, aliphatic, alicyclic, unsaturated, araliphatic, aromatic, substituted, or unsubstituted in nature. The molecular weight of the amine-terminated component for use in the invention may range from about 100 to about 10,000. In one embodiment, the amine-terminated component is about 500 or greater, preferably about 1000 or greater, and even more preferably about 2000 or greater. In another embodiment, the amine-terminated component molecular weight is about 8000 or less, preferably about 4,000 or less, and more preferably about 3,000 or less. For example, in one embodiment, the molecular weight of the amine-terminated component is about 1000 to about 4000. Because lower molecular weight amine-terminated components may be prone to forming solid polyurea prepolymer, a higher molecular weight oligomer may be used to avoid solid formation.

The amine-terminated component may be amine-terminated polyhydrocarbons including, but not limited to, amine-terminated polybutadiene, amine-terminated polyisoprene; poly(hydrogenated isoprene)amine; poly(hydrogenated butadiene)amine; and mixtures thereof. In particular, the hydroxy-terminated component preferably has two or more reactive amino groups per molecule, such as primary or secondary amino groups, and at least one conjugated diene hydrocarbon. The conjugated diene hydrocarbon may be unsubstituted, 2-substituted, or 2,3-disubstituted 1,3-dienes or 4 up to about 12 carbon atoms. In one embodiment, the diene has up to 6 carbon atoms and the substituents in the 2-

12

and/or 3-position may be H, alkyl, preferably lower alkyl, aryl, halogen, and mixtures thereof. The diene may be 1,3-butadiene, isoprene, 2-cyano-1,3-butadiene, 2,3-dimethyl-1,3-butadiene, 2-phenyl-1,3-butadiene, 2-methyl-3-phenyl-1,3-butadiene, and the like.

In one embodiment, the amine-terminated component includes amine-terminated polybutadiene (ATPB) where the functional amino groups are primary amino groups, secondary amino groups, or a combination thereof. The ATPB may have amino functionality of about 1.8 to about 3 per chain. In one embodiment, the amino functionality is about 2 to about 3 per chain. In another embodiment, the amino functionality of the ATPB is about 2.2 to about 2.6 per chain. Because the amino functionality has an effect on the viscosity during prepolymer preparation, in one embodiment, the amino functionality of the ATPB is about 2.0 to about 2.3 per chain. In fact, the use of a ATPB with lower amino functionality may alleviate the need for more isocyanate, which increases cost and handling issues, to reduce the viscosity.

Those of ordinary skill in the art would be aware of methods to prepare amine-terminated polybutadienes for use with the present invention. For example, ATPBs may be synthesized from functionalized initiators and butadiene monomer or by converting hydroxyl-terminated polybutadiene (HTPB) to ATPB by multi-step synthetic pathways. U.S. Pat. No. 4,658,062, the entire disclosure of which is incorporated by reference herein, discusses such methods. In addition, U.S. Pat. No. 4,994,621 discloses reacting liquid HTPB polymer with several oxirane units per hydroxyl group, to produce a secondary hydroxyl-terminated polymer containing ether linkages, which are then aminated by reacting ammonia with the hydroxyl groups under reducing conditions provided by hydrogen under pressure. Furthermore, ATPBs having one or two terminal amino groups may be prepared by cyanoalkylating a hydroxy-terminated polybutadiene by Michael addition of acrylonitrile in the presence of a base, forming nitrile termination, followed by hydrogenation in the presence of a Group VIII metal as catalyst. U.S. Pat. No. 6,831,136, the disclosure of which is incorporated by reference herein in its entirety, discusses such a method.

When a diisocyanate is reacted with an amine-terminated component of the present invention, long polymer chains are formed. A general reaction scheme between a diisocyanate and a amine-terminated component having primary amino groups according to the invention is as follows:



13

where  $n$  is the number of repeat units, i.e., about 1 or greater, and  $R$  and  $R_1$  are independently straight chains or branched hydrocarbon chains having about 1 to about 20 carbons, a phenyl group, or a mixture thereof.

In addition, when the amine-terminated component includes secondary amino groups, the reaction scheme is as follows:



where  $n$  is the number of repeat units, i.e., about 1 or greater, and  $R$  and  $R_1$  are independently straight chains or branched hydrocarbon chains having about 1 to about 20 carbons, a phenyl group, or a mixture thereof.

Furthermore, when the amine-terminated component includes a mixture of primary and secondary amine-terminated components, the reaction scheme is as follows:



where  $n$  is the number of repeat units, i.e., about 1 or greater, and  $R$  and  $R_1$  are independently straight chains or branched hydrocarbon chains having about 1 to about 20 carbons, a phenyl group, or a mixture thereof.

The amine-terminated component may be blended with other amine-terminated components including, but not limited to, amine-terminated hydrocarbons, amine-terminated polyethers, amine-terminated polyesters, amine-terminated polycarbonates, amine-terminated polycaprolactones, and mixtures thereof.

#### Hybrid Prepolymer

The prepolymer may also have both urethane and urea linkages. Such a prepolymer is distinct from a polyurethane prepolymer including only an isocyanate and a hydroxy-

14

terminated component or a polyurea prepolymer including only an isocyanate and an amine-terminated component. For the sake of clarity, this type of segment will be referred to as a hybrid prepolymer throughout the application.

For example, in one embodiment, the isocyanate-reactive component may have at least one terminal hydroxyl group and at least one terminal amino group. In particular, the iso-

cyanate-reactive component may have at least one conjugated diene hydrocarbon terminated at one end with a primary or secondary amino group and terminated at the other end with a primary or secondary hydroxyl group.

In this regard, the hybrid isocyanate-reactive component may have one of the following general formulas:



$R$ ,  $R_1$ , and  $R_2$  may independently be any alkyl group having from about 1 to about 20 carbon atoms, preferably about 1 to about 12 carbon atoms, a phenyl group, a cyclic group, or mixture thereof.  $X$  may be unsubstituted, 2-substituted, or 2,3-disubstituted 1,3-dienes or 4 up to about 12 carbon atoms

15

and n is the number of repeat units, i.e., about 1 or greater. In one embodiment, the diene has up to 6 carbon atoms and the substituents in the 2- and/or 3-position may be H, alkyl, preferably lower alkyl, aryl, halogen, and mixtures thereof. The diene may be 1,3-butadiene, isoprene, 2-cyano-1,3-butadiene, 2,3-dimethyl-1,3-butadiene, 2-phenyl-1,3-butadiene, 2-methyl-3-phenyl-1,3-butadiene, and the like.

16

When a diisocyanate is reacted with a hybrid isocyanate-reactive component of the present invention, long polymer chains are formed. A general reaction scheme between a diisocyanate and a hybrid isocyanate-reactive component having primary hydroxy and amino groups according to the invention is as follows:



30

where n is the number of repeat units, i.e., about 1 or greater, and R and R<sub>1</sub> are independently straight chains or branched hydrocarbon chains having about 1 to about 20 carbons, a phenyl group, or a mixture thereof.

35 In addition, when the hybrid isocyanate-reactive component includes a secondary hydroxy group and a primary amino group, the reaction scheme is as follows:



17

where  $n$  is the number of repeat units, i.e., about 1 or greater, and  $R$  and  $R_1$  are independently straight chains or branched hydrocarbon chains having about 1 to about 20 carbons, a phenyl group, or a mixture thereof.

Furthermore, when the hybrid isocyanate-reactive component includes a primary hydroxy group and a secondary amino group, the reaction scheme is as follows:



where  $n$  is the number of repeat units, i.e., about 1 or greater, and  $R$  and  $R_2$  are independently straight chains or branched hydrocarbon chains having about 1 to about 20 carbons, a phenyl group, or a mixture thereof.

Moreover, when the hybrid isocyanate-reactive component includes secondary hydroxyl and amino groups, the reaction scheme is as follows:



where  $n$  is the number of repeat units, i.e., about 1 or greater, and  $R$ ,  $R_1$ , and  $R_2$  are independently straight chains or branched hydrocarbon chains having about 1 to about 20 carbons, a phenyl group, or a mixture thereof.

#### Curative Blend

The prepolymers discussed above are cured with a curative blend that includes a curing agent(s) that promotes crosslinking of the hard segments in the prepolymer and a free radical initiator that promotes crosslinking of the soft segments in the polymer. In particular, the curing process involves the reaction of the prepolymer with an amine-terminated curing agent, a hydroxy-terminated curing agent, or a mixture thereof to crosslink the hard segments, i.e., the isocyanate groups and the amino and/or hydroxyl groups. In addition, elevated temperatures, infrared heat, and/or photoinitiators are used to initiate the free radical to crosslink the soft segments in the composition, i.e., the unsaturated portion of the elastomer.

In one embodiment, the curative blend includes at least one amine-terminated curing agent and a free radical initiator. In

18

another embodiment, the curative blend is a mixture of at least one hydroxy-terminated curing agent and a free radical initiator. In yet another embodiment, the curative blend includes at least one hydroxy-terminated curing agent, at least one amine-terminated curing agent, and a free radical initiator.

Furthermore, the curative blend may include a freezing point depressing agent to slow the onset of solidification.

Examples of freezing point depressing agents suitable for use in this aspect of the invention are disclosed in U.S. Patent Publication No. 2003/0212240, which is incorporated by reference herein in its entirety. In one embodiment, the freezing point depressing agent includes, but is not limited to, ethylene diamine, 1,3-diaminopropane, dimethylamino propylamine, tetraethylene pentamine, 1,2-propylenediamine, diethylami-

50 nopyrrolidine, 2,2,4-trimethyl-1,6-hexanediamine, 2,4,4-trimethyl-1,6-hexanediamine, and mixtures thereof.

#### Amine-Terminated Curing Agent

The prepolymers of the invention be cured with a single amine-terminated curing agent or a mixture of amine-terminated curing agents. Suitable amine-terminated curing agents include, but are not limited to, ethylene diamine; hexamethylene diamine; 1-methyl-2,6-cyclohexyl diamine; 2,2,4- and 2,4,4-trimethyl-1,6-hexanediamine; 4,4'-bis-(sec-butylamino)-dicyclohexylmethane and derivatives thereof; 1,4-bis-(sec-butylamino)-cyclohexane; 1,2-bis-(sec-butylamino)-cyclohexane; 4,4'-dicyclohexylmethane diamine; 1,4-cyclohexane-bis-(methylamine); 1,3-cyclohexane-bis-(methylamine), isomers, and mixtures thereof; diethylene glycol bis-(aminopropyl)ether; 2-methylpentamethylene-diamine; diaminocyclohexane, isomers, and mixtures thereof; diethylene triamine; triethylene tetramine; tetraethylene pentamine; propylene diamine; 1,3-diaminopropane; dimethylamino propylamine; diethylamino propylamine; imido-bis-(propylamine); monoethanolamine, diethanolamine;

triethanolamine; monoisopropanolamine, diisopropanolamine; isophoronediamine; 4,4'-methylenebis-(2-chloroaniline); 3,5-dimethylthio-2,4-toluenediamine; 3,5-dimethylthio-2,6-toluenediamine; 3,5-diethylthio-2,4-toluenediamine; 3,5-diethylthio-2,6-toluenediamine; 3,5-diethyltoluene-2,4-diamine; 3,5-diethyltoluene-2,6-diamine; 4,4'-bis-(sec-butylamino)-benzene; and derivatives thereof; 1,4-bis-(sec-butylamino)-benzene; 1,2-bis-(sec-butylamino)-benzene; N,N'-dialkylamino-diphenylmethane; trimethyleneglycol-di-p-aminobenzoate; polytetramethyleneoxide-di-p-aminobenzoate; 4,4'-methylenebis-(3-chloro-2,6-diethylenaniline); 4,4'-methylenebis-(2,6-diethylaniline); meta-phenylenediamine; paraphenylenediamine; N,N'-diisopropyl-isophoronediamine; polyoxypolyene diamine; propylene oxide-based triamine; 3,3'-dimethyl-4,4'-ciaminocyclohexylmethane; and mixtures thereof. In one embodiment, the amine-terminated curing agent is 4,4'-bis-(sec-butylamino)-dicyclohexylmethane.

The amine-terminated curing agent may have a molecular weight of about 64 or greater. In one embodiment, the molecular weight of the amine-curing agent is about 2000 or less. In addition, any of the amine-terminated moieties listed above for use as the isocyanate-reactive component to form the prepolymer may be used as curing agents to react with the prepolymers.

Of the list above, the saturated amine-terminated curing agents suitable for use with the present invention include, but are not limited to, ethylene diamine; hexamethylene diamine; 1-methyl-2,6-cyclohexyl diamine; 2,2,4- and 2,4,4-trimethyl-1,6-hexanediamine; 4,4'-bis-(sec-butylamino)-dicyclohexylmethane; 1,4-bis-(sec-butylamino)-cyclohexane; 1,2-bis-(sec-butylamino)-cyclohexane; derivatives of 4,4'-bis-(sec-butylamino)-dicyclohexylmethane; 4,4'-dicyclohexylmethane diamine; 1,4-cyclohexane-bis-(methylamine); 1,3-cyclohexane-bis-(methylamine); diethylene glycol bis(aminopropyl) ether; 2-methylpentamethylene-diamine; diaminocyclohexane; diethylene triamine; triethylene tetraamine; tetraethylene pentamine; propylene diamine; dipropylene triamine; 1,3-diaminopropane; dimethylamino propylamine; diethylamino propylamine; imido-bis(propylamine); monoethanolamine, diethanolamine; triethanolamine; monoisopropanolamine, diisopropanolamine; triisopropanolamine; isophoronediamine; N,N'-diisopropylisophorone diamine and mixtures thereof.

In one embodiment, the curative used with the prepolymer include 3,5-dimethylthio-2,4-toluenediamine, 3,5-dimethylthio-2,6-toluenediamine, 4,4'-bis-(sec-butylamino)-diphenylmethane, N,N'-diisopropyl-isophorone diamine; polyoxypolyene diamine; propylene oxide-based triamine; 3,3'-dimethyl-4,4'-ciaminocyclohexylmethane; and mixtures thereof.

Because unhindered primary diamines result in a rapid reaction between the isocyanate groups and the amine groups, in certain instances, a hindered secondary diamine may be more suitable for use in the prepolymer. Without being bound to any particular theory, it is believed that an amine with a high level of stearic hindrance, e.g., a tertiary butyl group on the nitrogen atom, has a slower reaction rate than an amine with no hindrance or a low level of hindrance. For example, 4,4'-bis-(sec-butylamino)-dicyclohexylmethane (Clearlink 1000) may be suitable for use in combination with an isocyanate to form the polyurea prepolymer. In addition, N,N'-diisopropyl-isophorone diamine, available from Huntsman Corporation under the tradename Jefflink, may be used as the secondary diamine curing agent.

In addition, a trifunctional curing agent can be used to help improve cross-linking and, thus, to further improve the shear resistance of the resulting polyurea elastomers. In one embodiment, a triol such as trimethylolpropane or a tetraol such as N,N,N',N'-tetrakis (2-hydroxylpropyl)ethylenediamine may be added to the formulations.

#### Hydroxy-Terminated Curing Agent

The prepolymers of the invention may also be cured with a single hydroxy-terminated curing agent or a mixture of hydroxy-terminated curing agents. Suitable hydroxy-terminated curing agents include, but are not limited to, ethylene glycol; diethylene glycol; polyethylene glycol; propylene glycol; 2-methyl-1,3-propanediol; 2-methyl-1,4-butanediol; dipropylene glycol; polypropylene glycol; 1,2-butanediol; 1,3-butanediol; 1,4-butanediol; 2,3-butanediol; 2,3-dimethyl-2,3-butanediol; trimethylolpropane; cyclohexyldimethylol; triisopropanolamine; N,N,N',N'-tetra-(2-hydroxypropyl)-ethylene diamine; diethylene glycol bis(aminopropyl)ether; 1,5-pentanediol; 1,6-hexanediol; 1,3-bis-(2-hydroxyethoxy)cyclohexane; 1,4-cyclohexyldimethylol; 1,3-bis-[2-(2-hydroxyethoxy)ethoxy]cyclohexane; 1,3-bis-[2-[2-(2-hydroxyethoxy)ethoxy]ethoxy]cyclohexane; polytetramethylene ether glycol, preferably having a molecular weight ranging from about 250 to about 3900; resorcinol-di-(beta-hydroxyethyl)ether and its derivatives; hydroquinone-di-(beta-hydroxyethyl)ether and its derivatives; 1,3-bis-(2-hydroxyethoxy)benzene; 1,3-bis-[2-(2-hydroxyethoxy)ethoxy]benzene; 1,3-bis-[2-[2-(2-hydroxyethoxy)ethoxy]ethoxy]benzene; N,N-bis(beta-hydroxypropyl)aniline; 2-propanol-1,1'-phenylaminobis; and mixtures thereof.

The hydroxy-terminated curing agent may have a molecular weight of at least about 50. In one embodiment, the molecular weight of the hydroxy-terminated curing agent is about 2000 or less. In yet another embodiment, the hydroxy-terminated curing agent has a molecular weight of about 250 to about 3900. It should be understood that molecular weight, as used herein, is the absolute weight average molecular weight and would be understood as such by one of ordinary skill in the art.

The saturated hydroxy-terminated curing agents, included in the list above, are preferred when making a light stable composition. Those saturated hydroxy-terminated curing agents include, but are not limited to, ethylene glycol; diethylene glycol; polyethylene glycol; propylene glycol; 2-methyl-1,3-propanediol; 2-methyl-1,4-butanediol; dipropylene glycol; polypropylene glycol; 1,2-butanediol; 1,3-butanediol; 1,4-butanediol; 2,3-butanediol; 2,3-dimethyl-2,3-butanediol; trimethylolpropane; cyclohexyldimethylol; triisopropanolamine; N,N,N',N'-tetra-(2-hydroxypropyl)-ethylene diamine; diethylene glycol bis-(aminopropyl)ether; 1,5-pentanediol; 1,6-hexanediol; 1,3-bis-(2-hydroxyethoxy)cyclohexane; 1,4-cyclohexyldimethylol; 1,3-bis-[2-(2-hydroxyethoxy)ethoxy]cyclohexane; 1,3-bis-[2-[2-(2-hydroxyethoxy)ethoxy]ethoxy]cyclohexane; polytetramethylene ether glycol having molecular weight ranging from about 250 to about 3900; and mixtures thereof

#### Free Radical Initiator

Free radicals promote crosslinking of the unsaturated segments of the prepolymer, i.e., the conjugated diene hydrocarbon. As such, any free radical initiator that generates free radicals is suitable for use in the curative blend. In one embodiment, a free radical initiator is included in the curative blend. One example of a suitable free radical initiator for use with the present invention is a peroxide. It should be further

understood that heat often facilitates initiation of the generation of free radicals when peroxides are used as a free-radical initiator.

The peroxide is not specifically limited, however, suitable peroxides include, but are not limited to, the following:



mixtures thereof. In addition, di-t-amyl peroxide, 1,1-bis(t-butylperoxy)-3,3,5-trimethylcyclohexane or 1,1-di(t-butylperoxy) 3,3,5-trimethyl cyclohexane, di-t-butyl peroxide, 2,5-di-(t-butylperoxy)-2,5-dimethyl hexane, 2,5-dimethyl-2,5-di-benzoylperoxyhexane, n-butyl-4,4-bis(t-butylperoxy) valerate, lauryl peroxide, benzoyl peroxide, t-butyl hydroperoxide, t-butyl cumylperoxide, t-butyl peroxybenzoate, 2,4-dichloro-benzoyl peroxide, and mixtures thereof are contemplated for use in curing the unsaturated soft segments in the prepolymer.

It is well known that peroxides are available in a variety of forms having different activity. The activity is typically defined by the percentage of pure peroxide in a mixture with an inert carrier. For example, DI-CUP® 40C, commercially available from GEO Specialty Chemicals of Gibbstown, N.J., is 40 percent active. The peroxide is typically present in an amount greater than about 0.1 parts per hundred of the composition, preferably about 0.1 to 15 parts per hundred of the composition, and more preferably about 0.2 to 5 parts per hundred of the composition. If the peroxide is present in pure form, it is preferably present in an amount of at least about 0.25 pph, more preferably between about 0.35 pph and about 2.5 pph, and most preferably between about 0.5 pph and about 2 pph per hundred of the composition. Peroxides are also available in diluted form, which are well-known to have differing activities, as described above. In this case, if diluted peroxides are employed in the present invention, one skilled in the art would know that the concentrations suitable for pure peroxides are easily adjusted for diluted peroxides by dividing by the activity. For example, 2 pph of a pure peroxide is equivalent 4 pph of a diluted peroxide that is 50 percent active (i.e., 2 divided by 0.5=4).

In addition to peroxides, other free radical initiators suitable for use with the present invention include persulfates, azo compounds, benzophenones, hydrazides, and combinations thereof are contemplated for use as part of the cure system for the dipolymer. In this aspect of the invention, the amount of free radical initiator is about 5 pph or less, preferably about 3 pph or less, more preferably about 2.5 pph or

less, and even more preferably about 2 pph or less per hundred of the composition. In still another embodiment, the amount of free radical initiator is about 1 pph or less, preferably about 0.75 pph or less per hundred of the composition.

5 Other Free Radical Initiators

Free radicals may be induced alternatively or additionally by one or more of an electron beam, UV or gamma radiation, x-rays, or any other high energy radiation source capable of generating free radicals.

10 For example, in one embodiment, the free radical initiator is UV radiation. In this aspect of the invention, the curative blend of the invention preferably includes at least one photoinitiator. In particular, when the curative blend includes at least one photoinitiator and the material is exposed to ultraviolet radiation, the dual cure may occur without heating the entire golf ball mold. For example, the photoinitiator is an ingredient that absorbs light and is responsible for the production of free radicals in a free radical polymerized system 15 such that the soft segments are crosslinked.

20 Suitable photoinitiators include, but are not limited to, 2,3-dimethoxy-2-phenylacetophenone, 2,2-diethoxyacetophenone, halogenated acetophenone derivatives, phenyl-bis(2,4,6-trimethylbenzoyl)phosphine oxide), 2-hydroxy-2-methylpropiophenone, benzophenone, diphenoxyl benzophenone, halogenated and amino functional benzophenones, 2-methylbenzophenone, alkyl ethers of benzoin, benzil dimethyl ketal, benzyl, 2-benzyl-2-N, N-dimethylamino-1-(4-morpholinophenyl)butanone, benzimidazoles, 25 anthraquinone derivatives, fluorenone derivatives, zanthone derivatives, thioxanthone derivatives, sulfonyl chlorides of aromatic compounds, camphorquinone, acylphosphine oxides, bis-acyl phosphine oxides, and mixtures thereof.

30 The photoinitiator(s) may be added to the curative blend such that it is present in an amount of about 0.05 to about 20 weight percent based on the total formulation. In one embodiment, the composition includes about 1 weight percent to about 10 weight percent photoinitiator based on the total weight of the composition. In another embodiment, the composition 35 includes about 2 weight percent to about 8 weight percent photoinitiator based on the total weight of the composition.

40 Forming the Compositions of the Invention

45 There are two basic techniques used to process the compositions of the invention: the one-shot technique and the prepolymer technique. The one-shot technique reacts the isocyanate-containing component and the isocyanate-reactive component, and the curative blend in one step, whereas the prepolymer technique requires a first reaction between the 50 isocyanate-reactive component(s) and an isocyanate to produce the prepolymer, and a subsequent reaction between the prepolymer and the curative blend. Either method may be employed to produce the compositions of the invention, however, the prepolymer technique is preferred because it provides better control of chemical reaction and, consequently, 55 results in more uniform properties for the elastomers.

In particular, whether the curative is a single amine-terminated curing agent and/or hydroxy-terminated curing agent and a free radical initiator or a mixture of amine-terminated 60 curing agent(s) and/or hydroxy-terminated curing agent(s) and a free radical initiator, once reacted with the prepolymer, the isocyanate (NCO) groups react with the hydroxy or amino groups to crosslink the hard segments in the prepolymer.

65 For example, when a urethane prepolymer reacts with a curing agent or curative blend including hydroxy-terminated components, the resulting polymer includes urethane linkages, as shown in the following general reaction scheme:



where n is the number of repeat units, i.e., about 1 or greater, X is a curing agent or curative blend including hydroxy groups, R and R<sub>2</sub> are independently straight chains or branched hydrocarbon chains having about 1 to about 20 carbons, a phenyl group, or a mixture thereof.

When a urea prepolymer reacts with a curing agent or curative blend including amine-terminated components, the resulting polymer includes urea linkages, as shown in the following general reaction scheme:



where n is the number of repeat units, i.e., about 1 or greater, X is a curing agent or curative blend including amino groups, R and R<sub>2</sub> are independently straight chains or branched hydrocarbon chains having about 1 to about 20 carbons, a phenyl group, or a mixture thereof.

When a hybrid prepolymer reacts with a curing agent or curative blend including hydroxy-terminated or amine-terminated components, the resulting polymer includes urea and urethane linkages, as shown in the following general reaction scheme:



where  $n$  is the number of repeat units, i.e., about 1 or greater,  $X$  is a curing agent or curative blend including hydroxy groups, amino groups, or combinations thereof,  $R$  and  $R_2$  are independently straight chains or branched hydrocarbon chains having about 1 to about 20 carbons, a phenyl group, or a mixture thereof.

Those of ordinary skill in the art would be aware of the similar general reaction schemes relating to the reaction between a urethane prepolymer and a curing agent or curative blend including amino groups and a urea prepolymer and a curing agent or curative blend including hydroxy groups. As discussed above, similar to a polymer resulting from the use of a hybrid prepolymer, the resulting polymer in these reactions will also include both urethane and urea linkages.

Because the curative blend also includes a free radical initiator, unlike conventional polyurethane and polyurea sys-

tems, the soft segments of the polymer are also crosslinked in the compositions of the present invention. There are several ways to accomplish the dual cure according to the present invention. However, it is important to note that regardless of 5 NCO content of the prepolymer, the dual cure of the present invention produces covers harder than covers formed with a single cure. For example, the hardness of a cover (as measured on the ball) of the invention may range from about 70 Shore C to about 100 Shore C. In one embodiment, the hardness of the cover is about 80 Shore C or greater. In another embodiment, the cover has a hardness of about 90 Shore C or greater.

The reaction scheme between a polyurethane prepolymer and a curative blend including hydroxy groups and a free radical initiator, such as an organic peroxide, is as follows:



where  $n$  is the number of repeat units, i.e., about 1 or greater, 40  $\text{XP}$  is a curative blend including hydroxy groups and an organic peroxide,  $R$  and  $R_2$  are independently straight chains or branched hydrocarbon chains having about 1 to about 20 carbons, a phenyl group, or a mixture thereof.

When a urea prepolymer reacts with a curing agent or curative blend including amino groups and a free radical initiator, such as an organic peroxide, the resulting polymer includes urea linkages, as shown in the following general reaction scheme:



where  $n$  is the number of repeat units, i.e., about 1 or greater, XP is a curative blend including amino groups and an organic peroxide, R and  $R_2$  are independently straight chains or branched hydrocarbon chains having about 1 to about 20 carbons, a phenyl group, or a mixture thereof.

When a hybrid prepolymer reacts with a curing agent or curative blend including hydroxy-terminated or amine-terminated components, the resulting polymer includes urea and urethane linkages, as shown in the following general reaction scheme:



where  $n$  is the number of repeat units, i.e., about 1 or greater, XP is a curative blend including hydroxy groups, amino groups, or combinations thereof, and an organic peroxide, R and  $R_2$  are independently straight chains or branched hydrocarbon chains having about 1 to about 20 carbons, a phenyl group, or a mixture thereof.

In one embodiment, the prepolymer and curative blend are mixed and poured into a mold. The temperature of the mold preferably ranges from about 100° F. to about 250° F. In one embodiment, the mold temperature ranges from about 120° F. to about 200° F. In another embodiment, the temperature of the mold ranges from about 140° F. to about 180° F. In still another embodiment, the mold temperature is about 150° F. to about 170° F.

The gel times preferably range from about 10 seconds to about 200 seconds. "Gel time" as used herein represents the amount of time, from the time the components are mixed to the time that the material is polymerized sufficiently that, if touched lightly with the edge of a metal spatula, no material adheres to the spatula, although the material is rubbery enough that an indentation in the material could easily and visibly be made. In contrast, "demold time" is the time at which the molded article is demolded without damage. In one embodiment, the gel time is from about 30 seconds to about 150 seconds. In another embodiment, the gel time is from about 40 seconds to about 130 seconds. In still another embodiment, the gel time is from about 45 seconds to about 120 seconds. Those of ordinary skill in the art are aware that the shorter gel times relate to higher NCO content. For example, a conventional polyurethane or polyurea composition with an NCO content of about 9 percent will typically result in a faster reaction rate and, thus, gel time of about 45 seconds.

However, the compositions of the present invention achieve the same gel time with less NCO content. For

example, the gel times above are achieved in the present invention with an NCO content of about 5 percent to 8 percent.

After a period of time, the mold temperature is elevated to initiate the free radical. In one embodiment, the period of time prior to elevation ranges from about 1 minute to about 30 minutes. In another embodiment, the period of time prior to elevation ranges from about 5 minutes to about 20 minutes, preferably about 8 minutes to about 15 minutes.

After the first stage of curing, a second stage occurs where the free radicals are initiated in order to effect cross-linking of the soft segments in the polymer. For example, the temperature may be elevated to any temperature that initiates the free radical for a predetermined amount of time. Without being bound to any particular theory, the hardness gradient may be manipulated through the use of a particular elevation temperature and/or time of exposure to the elevation temperature. 35 As such, the ranges herein are not limited and, instead, the inventors contemplate the use of various combinations of elevation temperatures and times in order to achieve a purposed hardness gradient according to the invention.

In one embodiment, the elevation temperature may range from about 250° F. to about 450° F., preferably from about 250° F. to about 400° F. In one embodiment, the elevation temperature may range from about 275° F. to about 400° F., preferably from about 275° F. to about 350° F. In another embodiment, the elevation temperature ranges from about 300° F. to about 330° F.

The period of time of exposure to the elevated temperature may be from about 2 minutes to about 20 minutes, preferably from about 4 minutes to about 15 minutes. In still another embodiment, the period of time of exposure to the elevated temperature is about 4 minutes or greater, preferably about 6 minutes or greater. In another embodiment, the material may be exposed to the elevated temperature for a time ranging from about 5 minutes to about 25 minutes, preferably about 8 minutes to about 20 minutes, and even more preferably about 12 minutes to about 18 minutes.

The second cure may also be effected through the use of infrared radiation, which may reduce or eliminate the need for conventional heating of the golf ball mold. As known to those 65 of ordinary skill in the art, IR radiation is a radiant form of heating in which objects and people are heated directly without the need to heat up the air in between. In particular, the IR

oven uses infrared radiation to provide high levels of temperatures (from less than 350° F. to about 2000° F.) to the surface and underlying mils of a golf ball layer. However, IR exposes the outer regions of the layer to a higher temperature than the inner regions of the layer creating a gradient. As such, the time of exposure and temperature of the oven will provide the depth and degree of curing.

At these NCO contents and gel times, the material hardness (as measured on buttons) preferably ranges from about 55 Shore D to about 85 Shore D or about 52 Shore C to about 100 Shore C. In one embodiment, the material hardness of the button is about 60 Shore D to about 80 Shore D or about 60 Shore C to about 90 Shore C. In another embodiment, the material hardness is about 62 Shore D or greater or about 85 Shore C or greater. In still another embodiment, the material hardness is about 64 Shore D or greater or about 90 Shore C or greater.

Similarly, the compression of solid spheres formed from the composition of the invention at the NCO content range and gel times defined above are preferably greater than 120 atti. In one embodiment, the compression range from about 120 atti to about 190 atti. In one embodiment, the compression is about 140 atti to about 180 atti. In yet another embodiment, the atti compression ranges from about 145 to about 180.

The COR of solid spheres formed from the compositions of the invention at the NCO content range and gel times defined above are preferably greater than about 0.570 at 125 ft/s. In one embodiment, the COR at 125 ft/s is about 0.580 or greater, preferably about 0.590 or greater, and more preferably about 0.600 or greater.

#### Blends

The compositions of the present invention may also be blended with other polymers. In particular, the compositions of the invention preferably include about 1 percent to about 100 percent of the crosslinked polyurethane/polyurea. In one embodiment, the compositions contain about 10 percent to about 90 percent of the crosslinked polyurethane/polyurea, preferably from about 10 percent to about 75 percent of the crosslinked polyurethane/polyurea, and about 90 percent to 10 percent, more preferably from about 90 percent to about 25 percent of the second polymer component and/or other materials as described below. For example, a blend in accordance in the present invention may have about 10 percent to about 40 percent of the crosslinked polyurethane/polyurea and about 60 percent to about 90 percent of another thermoplastic polymer, e.g. a conventional ionomer. In an alternate embodiment, a blend in accordance with the invention may include about 40 percent to about 80 percent of the crosslinked polyurethane/polyurea and about 20 percent to about 60 percent of another thermoplastic polymer. Unless otherwise stated herein, all percentages are given in percent by weight of the total composition of the golf ball layer in question.

For example, the compositions of the invention may be present in a blend with ionomeric copolymers or terpolymers, ionomeric precursors, thermoplastics, polyamides, polycarbonates, polyesters, polyurethanes, polyureas, thermoplastic elastomers, polybutadiene rubber, balata, grafted and non-grafted metallocene-catalyzed polymers, single-site polymers, high-crystalline acid polymers, cationic polymers, cationic and anionic urethane ionomers and urethane epoxies, polyurethane ionomers, polyurea ionomers, epoxy resins, polyethylenes, polyacrylin, siloxanes, and mixtures thereof.

Examples of suitable urethane ionomers are disclosed in U.S. Pat. No. 5,692,974, the disclosure of which is hereby incorporated by reference in its entirety. Other examples of suitable polyurethanes are described in U.S. Pat. No. 5,334,

673, the entire disclosure of which is incorporated by reference herein. Examples of suitable polyureas used to form the polyurea ionomer listed above are discussed in U.S. Pat. No. 5,484,870. In particular, the polyureas of U.S. Pat. No. 5,484,870 are prepared by reacting a polyisocyanate and a polyamine curing agent to yield polyurea, which are distinct from the polyureas of the present invention that are formed from a polyurea prepolymer and curing agent. Examples of suitable polyurethanes cured with epoxy group containing curing agents are disclosed in U.S. Pat. No. 5,908,358. The disclosures of the above patents are incorporated herein by reference in their entirety.

One of ordinary skill in the art would be well aware of methods to blend these polymeric materials with the organically modified silicate of the invention to form a composition for use in golf ball layers.

#### Additives

The compositions of the invention may include a variety of additives. For example, the compositions of the invention may be foamed by the addition of the at least one physical or chemical blowing or foaming agent. The use of a foamed polymer allows the golf ball designer to adjust the density or mass distribution of the ball to adjust the angular moment of inertia, and, thus, the spin rate and performance of the ball. Foamed materials also offer a potential cost savings due to the reduced use of polymeric material.

Blowing or foaming agents useful include, but are not limited to, organic blowing agents, such as azobisisformamide; azobisisobutyronitrile; diazoaminobenzene; N,N-dimethyl-N,N-dinitroso terephthalamide; N,N-dinitrosopentamethylene-tetramine; benzenesulfonyl-hydrazide; benzene-1,3-disulfonyl hydrazide; diphenylsulfon-3-3, disulfonyl hydrazide; 4,4'-oxybis benzene sulfonyl hydrazide; p-toluene sulfonyl semicarbazide; barium azodicarboxylate; butylamine nitrile; nitroureas; trihydrazino triazine; phenyl-methyl-uranthan; p-sulfonhydrazide; peroxides; and inorganic blowing agents such as ammonium bicarbonate and sodium bicarbonate. A gas, such as air, nitrogen, carbon dioxide, etc., can also be injected into the composition during the injection molding process.

Additionally, a foamed composition of the present invention may be formed by blending microspheres with the composition either during or before the molding process. Polymeric, ceramic, metal, and glass microspheres are useful in the invention, and may be solid or hollow and filled or unfilled. In particular, microspheres up to about 1000 micrometers in diameter are useful. Furthermore, the use of liquid nitrogen for foaming, as disclosed in U.S. Pat. No. 6,386,992, which is incorporated by reference herein, may produce highly uniform foamed compositions for use in the present invention.

Fillers may also be added to the compositions of the invention to affect Theological and mixing properties, the specific gravity (i.e., density-modifying fillers), the modulus, the tear strength, reinforcement, and the like. The fillers are generally inorganic, and suitable fillers include numerous metals, metal oxides and salts, such as zinc oxide and tin oxide, as well as barium sulfate, zinc sulfate, calcium carbonate, zinc carbonate, barium carbonate, clay, tungsten, tungsten carbide, an array of silicas, regrind (recycled core material typically ground to about 30 mesh particle), high-Mooney-viscosity rubber regrind, and mixtures thereof.

For example, the compositions of the invention can be reinforced by blending with a wide range of density-adjusting fillers, e.g., ceramics, glass spheres (solid or hollow, and filled or unfilled), and fibers, inorganic particles, and metal particles, such as metal flakes, metallic powders, oxides, and derivatives thereof, as is known to those with skill in the art.

The selection of such filler(s) is dependent upon the type of golf ball desired, i.e., one-piece, two-piece, multi-component, or wound, as will be more fully detailed below. Generally, the filler will be inorganic, having a density of greater than 4 g/cc, and will be present in amounts between about 5 and about 65 weight percent based on the total weight of the polymer components included in the layer(s) in question. Examples of useful fillers include zinc oxide, barium sulfate, calcium oxide, calcium carbonate, and silica, as well as other known corresponding salts and oxides thereof.

When the compositions of the invention are used in the core layers of the golf ball, fillers may also be used to modify the weight of the core to create a specialty ball, e.g., a lower weight ball is preferred for a player having a low swing speed.

Additional materials conventionally included in other golf ball compositions may also be included in the compositions of the invention. For example, antioxidants, stabilizers, softening agents, plasticizers, including internal and external plasticizers, reinforcing materials, and compatibilizers may also be added to any composition of the invention. Those of ordinary skill in the art are aware of the purpose of these additives and the amounts that should be employed to fulfill those purposes.

#### Golf Ball Construction

As discussed briefly above, the compositions of the present invention may be used with any type of ball construction including, but not limited to, one-piece, two-piece, three-piece, and four-piece designs, a double core, a double cover, an intermediate layer(s), a multilayer core, and/or a multi-layer cover depending on the type of performance desired of the ball. That is, the compositions of the invention may be used in a core, an intermediate layer, and/or a cover of a golf ball, each of which may have a single layer or multiple layers.

As used herein, the term "multilayer" means at least two layers. For instance, the core may be a one-piece core or a multilayer core, i.e., a core that has an innermost component with an additional core layer or additional core layers disposed thereon. As used herein, the terms "core" and "center" are generally used interchangeably to reference the innermost component of the ball. In some embodiments, however, the term "center" is used when there are multiple core layers, i.e., a center and an outer core layer.

When the golf ball of the present invention includes an intermediate layer, which may also include more than one layer, this layer may be incorporated with a single or multilayer cover, a single or multi-piece core, with both a single layer cover and core, or with both a multilayer cover and a multilayer core. The intermediate layer may be also be referred to as an inner cover layer or outer core layer, or any other layer(s) disposed between the inner core and the outer cover of a golf ball.

Referring to FIG. 1, a golf ball 2 of the present invention can include a center 4 and a cover 6 surrounding the center 4. While dimensions and materials are discussed in more detail below, a golf ball of the invention can include a large core, e.g., about 1.55 inches to about 1.60 inches, and a relatively soft, thin cover formed from the composition of the invention. In particular, the cover may have a thickness of about 0.02 inches to about 0.07 inches, preferably about 0.02 inches to about 0.045 inches, and more preferably about 0.025 inches to about 0.035 inches.

Referring to FIG. 2, a golf ball 8 of the present invention can include a center 10, a cover 14, and at least one intermediate layer 12 disposed between the cover and the center. In one embodiment, the intermediate layer 12 is formed from the composition of the invention. In another embodiment, the cover 14 is formed from the composition of the invention.

Each of the cover and center layers in FIG. 1 or 2 may include more than one layer, i.e., the golf ball can be a conventional three-piece wound ball, a two-piece ball, a ball having a multi-layer core and an intermediate layer or layers, etc.

Also, FIG. 3 shows a golf ball 16 of the present invention including a large core 18, a cover 22, and an inner cover layer 20. In one embodiment, the core 18 includes a center and an outer core layer. The inner cover layer 20 and/or cover 22 may be formed from the composition of the invention. In one embodiment, the inner cover layer 20 is formed from the composition of the invention and the cover 22 is formed from a polyurethane or polyurea material. In another embodiment, the cover 22 is formed from the composition of the invention.

In another embodiment, as shown in FIG. 4, a golf ball 24 of the present invention can include a large core having a center 26 and an intermediate layer 28 disposed underneath a dual cover having an inner cover layer 30 and an outer cover layer 32. The inner cover layer 30 and/or outer cover layer 32 is formed from the compositions of the invention. In one embodiment, the outer cover layer 32 is formed from the compositions of the invention. Further, any of the figures detailed herein may include embodiments wherein an optional wound layer is disposed between the center and the core of the golf ball.

Other non-limiting examples of suitable types of ball constructions that may be used with the present invention include those described in U.S. Pat. Nos. 6,056,842, 5,688,191, 5,713,801, 5,803,831, 5,885,172, 5,919,100, 5,965,669, 5,981,654, 5,981,658, and 6,149,535, as well as in Publication Nos. US2001/0009310 A1, US2002/0025862, and US2002/0028885. The entire disclosures of these patents and published patent applications are incorporated by reference herein.

#### Golf Ball Core Layer(s)

The cores of the golf balls formed according to the invention may be solid, semi-solid, hollow, fluid-filled or powder-filled, one-piece or multi-component cores. As used herein, the term "fluid" includes a liquid, a paste, a gel, a gas, or any combination thereof; the term "fluid-filled" includes hollow centers or cores; and the term "semi-solid" refers to a paste, a gel, or the like.

The core may have a diameter of about 1.5 inches to about 1.62 inches and the cover layer thickness may range from about 0.03 inches to about 0.06 inches. The core compression preferably ranges from about 30 to about 120 atti and the overall ball compression is about 50 to about 110.

Any core material known to one of ordinary skill in that art is suitable for use in the golf balls of the invention. Suitable core materials include thermoset materials, such as rubber, styrene butadiene, polybutadiene, isoprene, polyisoprene, trans-isoprene, as well as thermoplastics such as ionomer resins, polyamides or polyesters, and thermoplastic and thermoset polyurethane elastomers. For example, butadiene rubber, which, in an uncured state, typically has a Mooney viscosity (measured according to ASTM D1646-99) greater than about 20, preferably greater than about 30, and more preferably greater than about 40, may be used in one or more core layers of the golf balls prepared according to the present invention. In addition, the compositions of the invention may be incorporated the core.

A free-radical source, often alternatively referred to as a free-radical initiator, may optionally be used in the core, or one or more layers of the golf balls according to the invention, particularly when a polymer component includes a thermoset material. The free radical source for is preferably a peroxide, more preferably an organic peroxide. The peroxide is typi-

cally present in an amount greater than about 0.1 parts per hundred of the total polymer component, preferably about 0.1 to 15 parts per hundred of the polymer component, and more preferably about 0.2 to 5 parts per hundred of the total polymer component. It should be understood by those of ordinary skill in the art that the presence of certain components may require a larger amount of free-radical source than the amounts described herein. The free radical initiator may alternatively or additionally be one or more of an electron beam, UV or gamma radiation, x-rays, or any other high energy radiation source capable of generating free radicals. It should be further understood that heat often facilitates initiation of the generation of free radicals when peroxides are used as a free radical initiator.

#### Golf Ball Intermediate Layer(s)

When the golf ball of the present invention includes an intermediate layer, such as an inner cover layer or outer core layer, i.e., any layer(s) disposed between the inner core and the outer cover of a golf ball, this layer may be formed from the composition of the invention. For example, an intermediate layer or inner cover layer having a thickness of about 0.015 inches to about 0.06 inches may be disposed about a core. In this aspect of the invention, the core, which has a diameter ranging from about 1.5 inches to about 1.59 inches, may also be formed from a composition of the invention or, in the alternative, from a conventional rubber composition. The inner ball may be covered by a castable thermoset or injection moldable thermoplastic material or any of the other cover materials discussed below. In this aspect of the invention, the cover may have a thickness of about 0.02 inches to about 0.045 inches, preferably about 0.025 inches to about 0.04 inches. The core compression is about 30 to about 110 atti, preferably about 50 to about 100 atti, and the overall ball compression preferably ranges from about 50 to about 100 atti.

When not formed from the composition of the invention, the intermediate layer may be formed from a number of thermoplastic and thermosetting materials. For example, the intermediate layer(s) may be formed, at least in part, from one or more homopolymeric or copolymeric materials, such as ionomers, primarily or fully non-ionomeric thermoplastic materials, vinyl resins, polyolefins, polyurethanes, polyureas, such as those disclosed in U.S. Pat. No. 5,484,870, polyamides, acrylic resins and blends thereof, olefinic thermoplastic rubbers, block copolymers of styrene and butadiene, isoprene or ethylene-butylene rubber, copoly(ether-amide), such as PEBAK, sold by Arkema, Inc. of Philadelphia, Pa., polyphenylene oxide resins or blends thereof, and thermoplastic polyesters.

For example, the intermediate layer may be formed of low acid ionomers, such as those described in U.S. Pat. Nos. 6,506,130 and 6,503,156, high acid ionomers, highly neutralized polymers, such as those disclosed in U.S. Patent Publication Nos. 2001/0018375 and 2001/0019971, or mixtures thereof. The intermediate layer may also be formed from the compositions as disclosed in U.S. Pat. No. 5,688,191. The entire disclosures of these patents and publications are incorporated herein by express reference thereto.

The intermediate layer may also include a wound layer formed from a tensioned thread material. The thread may be single-ply or may include two or more plies. Suitable thread materials include, but are not limited to, fiber, glass, carbon, polyether urea, polyether block copolymers, polyester urea, polyester block copolymers, syndiotactic- or isotactic-poly(propylene), polyethylene, polyamide, poly(oxymethylene), polyketone, poly(ethylene terephthalate), poly(p-phenylene terephthalamide), poly(acrylonitrile), diaminodicyclohexyl-

methane, dodecanedicarboxylic acid, natural rubber, polyisoprene rubber, styrene-butadiene copolymers, styrene-propylene-diene copolymers, another synthetic rubber, or block, graft, random, alternating, brush, multi-arm star, branched, or dendritic copolymers, or mixtures thereof. Those of ordinary skill in the art are aware of the process for producing thread materials for use with the present invention.

#### Golf Ball Cover Layer(s)

The cover provides the interface between the ball and a club. Properties that are desirable for the cover are good 10 moldability, high abrasion resistance, high impact resistance, high tear strength, high resilience, and good mold release, among others. The cover layer may be formed, at least in part, from a composition of the invention. For example, the present 15 invention contemplates a golf ball having a large core of polybutadiene and a thin cover formed from the composition of the invention.

When the compositions of the invention are incorporated 20 into a core or intermediate/inner cover layer, however, the cover may be formed from one or more homopolymeric or 25 copolymeric materials as discussed in the section above pertaining to the intermediate layer. The cover may also be at least partially formed from a polybutadiene reaction product, as discussed above with respect to the core. Golf balls according to the invention may also be formed having a cover of polyurethane, polyurea, and polybutadiene materials discussed in U.S. Pat. No. 6,835,794.

For example, the cover may be formed from the reaction 30 product of an isocyanate and a hydroxy-terminated component that is cured with a curing agent to form a polyurethane. In another embodiment, the cover is formed from a reaction product of an isocyanate and an amine-terminated component that is cured with a curing agent to form a polyurea.

#### Layer Formation

The golf balls of the invention may be formed using a 35 variety of application techniques such as compression molding, flip molding, injection molding, retractable pin injection molding, reaction injection molding (RIM), liquid injection molding (LIM), casting, vacuum forming, powder coating, flow coating, spin coating, dipping, spraying, and the like. Conventionally, compression molding and injection molding 40 are applied to thermoplastic materials, whereas RIM, liquid injection molding, and casting are employed on thermoset materials. These and other manufacture methods are disclosed in U.S. Pat. Nos. 6,207,784 and 5,484,870, the disclosures of which are incorporated herein by reference in their 45 entirety.

Cores of the golf balls of the invention may be formed by 50 any suitable method known to those of ordinary skill in art. When the cores are formed from a thermoset material, compression molding is a particularly suitable method of forming the core. In a thermoplastic core embodiment, on the other hand, the cores may be injection molded. Furthermore, U.S. Pat. Nos. 6,180,040 and 6,180,722 disclose methods of preparing dual core golf balls. The disclosures of these patents 55 are hereby incorporated by reference in their entirety.

The intermediate layer and/or cover layer may also be formed using any suitable method known to those of ordinary 60 skill in the art. For example, an intermediate layer may be formed by blow molding and covered with a dimpled cover layer formed by injection molding, compression molding, casting, vacuum forming, powder coating, and the like.

The use of various dimple patterns and profiles provides a 65 relatively effective way to modify the aerodynamic characteristics of a golf ball. As such, the manner in which the dimples are arranged on the surface of the ball can be by any available method. For instance, the ball may have an icosa-

hedron-based pattern, such as described in U.S. Pat. No. 4,560,168, or an octahedral-based dimple patterns as described in U.S. Pat. No. 4,960,281. Furthermore, the resultant golf balls prepared according to the invention typically will have dimple coverage greater than about 60 percent, preferably greater than about 65 percent, and more preferably greater than about 70 percent.

#### Golf Ball Post-Processing

The golf balls of the present invention may be painted, coated, or surface treated for further benefits. For example, golf balls may be coated with urethanes, urethane hybrids, ureas, urea hybrids, epoxies, polyesters, acrylics, or combinations thereof in order to obtain an extremely smooth, tack-free surface. If desired, more than one coating layer can be used. The coating layer(s) may be applied by any suitable method known to those of ordinary skill in the art. In one embodiment, the coating layer(s) is applied to the golf ball cover by an in-mold coating process, such as described in U.S. Pat. No. 5,849,168, which is incorporated in its entirety by reference herein.

Any of the golf ball layers may be surface treated by conventional methods including blasting, mechanical abrasion, corona discharge, plasma treatment, and the like, and combinations thereof. In fact, because low surface energy, or surface tension, is a key feature of polysiloxanes, layers formed from the compositions of the invention may be surface treated according to U.S. Patent Publication No. 2003/0199337, the disclosure of which is incorporated in its entirety by reference herein.

#### Golf Ball Properties

The properties such as core diameter, intermediate layer and cover layer thickness, hardness, and compression have been found to effect play characteristics such as spin, initial velocity and feel of the present golf balls.

#### Component Dimensions

Dimensions of golf ball components, i.e., thickness and diameter, may vary depending on the desired properties. For the purposes of the invention, any layer thickness may be employed. For example, the present invention relates to golf balls of any size, although the golf ball preferably meets USGA standards of size and weight. While "The Rules of Golf" by the USGA dictate specifications that limit the size of a competition golf ball to more than 1.680 inches in diameter, golf balls of any size can be used for leisure golf play. The preferred diameter of the golf balls is from about 1.680 inches to about 1.800 inches. The more preferred diameter is from about 1.680 inches to about 1.760 inches. A diameter of from about 1.680 inches (43 mm) to about 1.740 inches (44 mm) is most preferred, however diameters anywhere in the range of from 1.700 to about 1.950 inches can be used.

Preferably, the overall diameter of the core and all intermediate layers is about 80 percent to about 98 percent of the overall diameter of the finished ball. The core may have a diameter ranging from about 0.09 inches to about 1.65 inches. In one embodiment, the diameter of the core of the present invention is about 1.2 inches to about 1.630 inches. For example, when part of a two-piece ball according to invention, the core may have a diameter ranging from about 1.5 inches to about 1.62 inches. In another embodiment, the diameter of the core is about 1.3 inches to about 1.6 inches, preferably from about 1.39 inches to about 1.6 inches, and more preferably from about 1.5 inches to about 1.6 inches. In yet another embodiment, the core has a diameter of about 1.55 inches to about 1.65 inches, preferably about 1.55 inches to about 1.60 inches. In one embodiment, the core diameter is about 1.59 inches or greater. In another embodiment, the diameter of the core is about 1.64 inches or less.

When the core includes an inner core layer and an outer core layer, the inner core layer is preferably about 0.5 inches or greater and the outer core layer preferably has a thickness of about 0.1 inches or greater. For example, when part of a multi-layer ball according to invention, the center may have a diameter ranging from about 0.5 inches to about 1.30 inches and the outer core layer may have a diameter ranging from about 0.12 inches to about 0.5 inches. In one embodiment, the inner core layer has a diameter from about 0.09 inches to about 1.2 inches and the outer core layer has a thickness from about 0.1 inches to about 0.8 inches. In yet another embodiment, the inner core layer diameter is from about 0.095 inches to about 1.1 inches and the outer core layer has a thickness of about 0.20 inches to about 0.03 inches.

The cover typically has a thickness to provide sufficient strength, good performance characteristics, and durability. In one embodiment, the cover thickness is from about 0.02 inches to about 0.12 inches, preferably about 0.1 inches or less. For example, when part of a two-piece ball according to invention, the cover may have a thickness ranging from about 0.03 inches to about 0.09 inches. In another embodiment, the cover thickness is about 0.05 inches or less, preferably from about 0.02 inches to about 0.05 inches, and more preferably about 0.02 inches and about 0.045 inches.

The range of thicknesses for an intermediate layer of a golf ball is large because of the vast possibilities when using an intermediate layer, i.e., as an outer core layer, an inner cover layer, or a moisture/vapor barrier layer. When used in a golf ball of the invention, the intermediate layer, or inner cover layer, may have a thickness about 0.3 inches or less. In one embodiment, the thickness of the intermediate layer is from about 0.002 inches to about 0.1 inches, preferably about 0.01 inches or greater. For example, when part of a three-piece ball or multi-layer ball according to invention, the intermediate layer and/or inner cover layer may have a thickness ranging from about 0.015 inches to about 0.06 inches. In another embodiment, the intermediate layer thickness is about 0.05 inches or less, more preferably about 0.01 inches to about 0.045 inches.

#### 40 Hardness

Because the compositions of the invention may be used in any layer of a golf ball, the golf ball construction, physical properties, and resulting performance may vary greatly depending on the layer(s) of the ball that include the compositions of the invention.

The cores included in golf balls of the present invention may have varying hardnesses depending on the particular golf ball construction. In one embodiment, the core hardness is at least about 15 Shore A, preferably about 30 Shore A, as measured on a formed sphere. In another embodiment, the core has a hardness of about 50 Shore A to about 90 Shore D. In yet another embodiment, the hardness of the core is about 80 Shore D or less. Preferably, the core has a hardness about 30 to about 65 Shore D, and more preferably, the core has a hardness about 35 to about 60 Shore D. For example, when a core is formed from the composition of the invention, the core may have a hardness of about 40 Shore to about 50 Shore D.

The intermediate layer(s) of the present invention may also vary in hardness depending on the specific construction of the ball. In one embodiment, the hardness of the intermediate layer is about 30 Shore D or greater. In another embodiment, the hardness of the intermediate layer is about 90 Shore D or less, preferably about 80 Shore D or less, and more preferably about 70 Shore D or less. For example, when an intermediate layer is formed from the composition of the invention, the hardness of the intermediate layer may be about 65 Shore D or less, preferably ranging from about 35 Shore D to about 60

Shore D. In yet another embodiment, the hardness of the intermediate layer is about 50 Shore D or greater, preferably about 55 Shore D or greater. In one embodiment, the intermediate layer hardness is from about 55 Shore D to about 65 Shore D. The intermediate layer may also be about 65 Shore D or greater. For example, a golf ball of the invention may include an inner cover formed from a rosin-modified polymeric composition of the invention having a hardness of about 60 Shore D to about 75 Shore D.

As with the core and intermediate layers, the cover hardness may vary depending on the construction and desired characteristics of the golf ball. The ratio of cover hardness to inner ball hardness is a primary variable used to control the aerodynamics of a ball and, in particular, the spin of a ball. In general, the harder the inner ball, the greater the driver spin and the softer the cover, the greater the driver spin.

For example, when the intermediate layer is intended to be the hardest point in the ball, e.g., about 60 Shore D to about 75 Shore D, the cover material may have a hardness of about 20 Shore D or greater, preferably about 25 Shore D or greater, and more preferably about 30 Shore D or greater, as measured on the slab. In another embodiment, the cover itself has a hardness of about 30 Shore D or greater. In particular, the cover may be from about 30 Shore D to about 70 Shore D. In one embodiment, the cover has a hardness of about 40 Shore D to about 65 Shore D, and in another embodiment, about 40 Shore to about 55 Shore D. In another aspect of the invention, the cover has a hardness less than about 45 Shore D, preferably less than about 40 Shore D, and more preferably about 25 Shore D to about 40 Shore D. In one embodiment, the cover has a hardness from about 30 Shore D to about 40 Shore D.

In one embodiment, the cover hardness is about 60 Shore D or greater. In another embodiment, the cover hardness is about 62 Shore D or greater. In still another embodiment, the cover hardness is about 64 Shore D or greater. For example, the cover hardness may range from about 55 Shore D to about 85 Shore D. In another embodiment, the cover hardness is about 60 Shore D to about 80 Shore D. This range of hardness may be used in a 2-piece ball, i.e., a ball with a core and a cover, as well as a multilayer ball, e.g., a ball with one or more intermediate layers disposed between the core and the cover.

When used in any layer of a golf ball, the compositions of the invention produce a hardness gradient of at least about 5 percent from a first point on the inner surface of the layer to a second point on the outer surface of the layer. For example, FIG. 5a illustrates a golf ball 34 having a cover 38 with a first hardness at point A (an interior location), a second hardness at point B (a location between point A and point C), and a third hardness at point C (an exterior location). The hardness at point B is preferably greater than the hardness at point A and less than the hardness at point C.

In one embodiment, the hardness at point A is about 90 percent of the hardness of point C. In another embodiment, the hardness at point A is about 85 percent of the hardness of point C. In yet another embodiment, the hardness at point A is about 80 percent of the hardness of point C. In still another embodiment, the hardness at point A is about 75 percent of the hardness of point C.

In other words, the hardness at point C may be greater than the hardness at point A by about 5 percent to about 40 percent. In one embodiment, the hardness at point C is about 110 percent or greater of the hardness at point A. In another embodiment, the hardness at point C is greater than the hardness at point A by about 8 percent to about 35 percent, preferably about 12 percent to about 30 percent. In yet another embodiment, the hardness at point C is about 120 percent or greater of the hardness at point A.

In one embodiment, the hardness at point B may be about 102 percent to about 108 percent of the hardness of point A. In another embodiment, point B may have a hardness about 105 percent to about 115 percent of the hardness at point A.

5 The hardness gradient between point A and point C may range from about 1 percent to about 45 percent. In one embodiment, the hardness gradient is about 5 percent to about 40 percent. In another embodiment, the hardness gradient is about 10 percent to about 35 percent. In still another embodiment, the hardness gradient is about 12 percent to about 33 percent. In yet another embodiment, the hardness gradient is about 20 percent or greater, preferably about 25 percent to about 35 percent.

10 When measured on buttons, such as the button shown in FIG. 5b, the hardness at point A may range from about 50 Shore C to about 70 Shore C. In one embodiment, the point A hardness is about 55 Shore C or greater. In another embodiment, the Shore C hardness at point A is about 58 or greater. 15 In still another embodiment, the Shore C hardness at point A is about 59 or greater. The hardness at point C is about 52 Shore C to about 100 Shore C. In one embodiment, the hardness at point C is about 60 Shore C to about 95 Shore C. In another embodiment, the Shore C hardness at point C is about 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9

## Coefficient of Restitution

The present invention contemplates golf balls having CORs from about 0.700 to about 0.850 at an inbound velocity of about 125 ft/sec. In one embodiment, the COR is about 0.750 or greater, preferably about 0.780 or greater. In another embodiment, the ball has a COR of about 0.800 or greater. In yet another embodiment, the COR of the balls of the invention is about 0.800 to about 0.815.

Alternatively, the maximum COR of the ball is one that does not cause the golf ball to exceed initial velocity requirements established by regulating entities such as the USGA. As used herein, the term "coefficient of restitution" (CoR) is calculated by dividing the rebound velocity of the golf ball by the incoming velocity when a golf ball is shot out of an air cannon. The COR testing is conducted over a range of incoming velocities and determined at an inbound velocity of 125 ft/s. Another measure of this resilience is the "loss tangent," or  $\tan \delta$ , which is obtained when measuring the dynamic stiffness of an object. Loss tangent and terminology relating to such dynamic properties is typically described according to ASTM D4092-90. Thus, a lower loss tangent indicates a higher resiliency, thereby indicating a higher rebound capacity. Low loss tangent indicates that most of the energy imparted to a golf ball from the club is converted to dynamic energy, i.e., launch velocity and resulting longer distance. The rigidity or compressive stiffness of a golf ball may be measured, for example, by the dynamic stiffness. A higher dynamic stiffness indicates a higher compressive stiffness. To produce golf balls having a desirable compressive stiffness, the dynamic stiffness of the crosslinked material should be less than about 50,000 N/m at  $-50^\circ$  C. Preferably, the dynamic stiffness should be between about 10,000 and 40,000 N/m at  $-50^\circ$  C., more preferably, the dynamic stiffness should be between about 20,000 and 30,000 N/m at  $-50^\circ$  C.

## Moisture Vapor Transmission

The moisture vapor transmission of a golf ball portion formed from the compositions of the invention may be expressed in terms of absorption, e.g., weight gain or size gain over a period of time at a specific conditions, and transmission, e.g., moisture vapor transmission rate (MVTR) according to ASTM E96-00. MVTR refers to the mass of water vapor that diffused into a material of a given thickness per unit area per unit time at a specific temperature and humidity differential. For example, weight changes of a golf ball portion monitored over a period of seven weeks in 100 percent relative humidity and  $72^\circ$  F. help to demonstrate which balls have better water resistance.

In one embodiment, the golf ball portions of the invention have a weight gain of about 15 grams per 100 in<sup>2</sup> per day or less at  $38^\circ$  C. and 90 percent relative humidity. In another embodiment, the golf balls of the invention have a weight gain of about 12.5 grams per 100 in<sup>2</sup> per day or less. In still another embodiment, the weight gain of the golf balls of the invention is about 7 grams per 100 in<sup>2</sup> per day or less. In yet another embodiment, the weight gain is about 5 grams per 100 in<sup>2</sup> per day or less. The golf balls of the invention preferably have a weight gain of about 3 grams per 100 in<sup>2</sup> per day or less.

Size gain may also be used as an indicator of water resistance. That is, the more water a golf ball takes on, the larger

golf ball becomes due to the water enclosed beneath the outermost layer of the golf ball portion. Thus, the golf balls of the invention preferably have no appreciable size gain. In one embodiment, the size gain of the golf balls of the invention after a seven-week period is about 0.001 inches or less.

## EXAMPLES

The following examples are only representative of the methods and materials for use in golf ball compositions and golf balls of this invention, and are not to be construed as limiting the scope of the invention in any way.

## Example 1

## Compositions According to the Invention

Compositions were formed according to the invention as shown below in Table 1. In particular, Curative A is a curative blend of the invention and Curative B is a conventional curative blend.

TABLE 1

|                         | Formulation #1 | Control A |
|-------------------------|----------------|-----------|
| Prepolymer <sup>1</sup> | 1 eq.          | 1 eq.     |
| Curative A <sup>2</sup> | 0.95 eq.       | 0.95 eq.  |
| Curative B <sup>3</sup> |                |           |
| White Dispersion        | 1%             | 1%        |

<sup>1</sup>Prepolymer is a reaction product of H<sub>12</sub>MDI and Krasol ® LBH 2000 from Sartomer, which is a linear polybutadiene with a molecular weight of 2000 and hydroxy end groups.

<sup>2</sup>Curative A is a mixture of 0.475 eq. Ethacure ® 300 from Albemarle Corporation, which is dimethylthiobutene diamine with a molecular weight of 214, and 0.475 eq. Unilink ® 4200, which is a secondary aromatic diamine with a molecular weight of 310 and 1 percent dicumyl peroxide.

<sup>3</sup>Curative B is a mixture of 0.475 eq. Ethacure ® 300 from Albemarle Corporation, which is dimethylthiobutene diamine with a molecular weight of 214, and 0.475 eq. Unilink ® 4200, which is a secondary aromatic diamine with a molecular weight of 310.

Formulation #1 and Control A were prepared at varying concentrations of NCO ranging from about 5 percent to about 9 percent, as shown below in Table 2.

TABLE 2

| % NCO<br>(seconds) | Gel Time | Formulation #1 |   |   |   |   | Control A |   |   |   |   |
|--------------------|----------|----------------|---|---|---|---|-----------|---|---|---|---|
|                    |          | A              | B | C | D | E | 1         | 2 | 3 | 4 | 5 |
| 5.12               | 120      | ✓              |   |   |   |   |           | ✓ |   |   |   |
| 6.07               | 100      |                | ✓ |   |   |   |           |   | ✓ |   |   |
| 7.13               | 75       |                |   | ✓ |   |   |           |   |   | ✓ |   |
| 8.00               | 60       |                |   |   | ✓ |   |           |   |   | ✓ |   |
| 8.88               | 45       |                |   |   |   | ✓ |           |   |   |   | ✓ |

The prepolymer and curative were mixed in a FlackTek high speed mixer and poured into a  $160^\circ$  F. mold. The mold was then placed into a Carver press at 20,000 psi and heating continued for 12 minutes. In the case of the formulations of the invention, i.e., Formulations #1A, #1B, #1C, #1D, and #1E, the press temperature was then raised to  $325^\circ$  F. and the formulations were cured for an additional 15 minutes resulting in 1.620 solid spheres. Data was obtained using the spheres and material hardness buttons.

As shown in Table 3 below, the formulations of the invention result in higher hardness, compression, and COR values as compared to conventional formulations at the same NCO content and gel time.

TABLE 3

|                | Formulation #1 |       |       |       |       | Control A |       |       |       |       |
|----------------|----------------|-------|-------|-------|-------|-----------|-------|-------|-------|-------|
|                | A              | B     | C     | D     | E     | 1         | 2     | 3     | 4     | 5     |
| Compression    | 148            | 162   | 169   | 175   | 178   | 16        | 63    | 90    | 104   | 114   |
| Shore C        | 90             | 92    | 94    | 94    | 95    | 62        | 71    | 76    | 78    | 80    |
| Shore D        | 64             | 67    | 73    | 76    | 78    | 40        | 47    | 52    | 55    | 57    |
| COR @ 125 ft/s | 0.600          | 0.659 | 0.667 | 0.720 | 0.738 | 0.500     | 0.516 | 0.540 | 0.553 | 0.565 |

In sum, the formulations of the invention deliver higher material hardness without increasing NCO content, thus, allowing manageable reaction rates.

Example 2

Dual Cured Buttons Formed from Compositions of the Invention

Compositions were formed according to the invention. In particular, the prepolymer is a reaction product of H<sub>12</sub>MDI and Krasol® LBH 2000 from Sartomer, which is a linear polybutadiene with a molecular weight of 2000 and hydroxy end groups. The curative is a mixture of 0.475 eq. Ethacure® 300 from Albemarle Corporation, which is dimethylthiobutene diamine with a molecular weight of 214, and 0.475 eq. Unilink® 4200, which is a secondary aromatic diamine with a molecular weight of 310 and 1 percent dicumyl peroxide.

The compositions were subjected to various degrees of curing. In particular, the control button was subjected to a single cure, i.e., no elevated temperature to initiate the free radical. In contrast, after the initial cure, Invention #1 button was placed between two platens, one at room temperature and the other at 400° F. for four (4) minutes. Invention #2 button was subjected to the same cure process for six (6) minutes. As shown below in Table 4 and according to the hardness points according to FIG. 5b, the control had a constant hardness throughout the button, whereas Invention #1 Button had a hardness gradient of about 12 percent and Invention #2 Button had a hardness gradient of about 30 percent.

TABLE 4

|                       | Single Cure<br>(Control) | Invention #1 Button<br>(Dual Cure (4 min.)) | Invention #1 Button<br>(Dual Cure (6 min.)) |
|-----------------------|--------------------------|---------------------------------------------|---------------------------------------------|
| Hardness<br>(Point A) | 59 Shore C               | 59 Shore C                                  | 59 Shore C                                  |
| Hardness<br>(Point C) | 59 Shore C               | 66 Shore C                                  | 77 Shore C                                  |
| Gradient              | 0                        | 11.8%                                       | 30.5%                                       |

Thus, both the elevation temperature and time period of exposure to the elevation temperature affects the hardness gradient.

Other than in the operating examples, or unless otherwise expressly specified, all of the numerical ranges, amounts, values and percentages such as those for amounts of materials, times and temperatures of reaction, ratios of amounts, values for molecular weight (whether number average molecular weight ("Mn") or weight average molecular weight ("Mw")), and others in the following portion of the specification may be read as if prefaced by the word "about" even though the term "about" may not expressly appear with the value, amount or range. Accordingly, unless indicated to the contrary, the numerical parameters set forth in the following specification and attached claims are approximations that

may vary depending upon the desired properties sought to be obtained by the present invention. At the very least, and not as an attempt to limit the application of the doctrine of equivalents to the scope of the claims, each numerical parameter should at least be construed in light of the number of reported significant digits and by applying ordinary rounding techniques.

Notwithstanding that the numerical ranges and parameters setting forth the broad scope of the invention are approximations, the numerical values set forth in the specific examples are reported as precisely as possible. Any numerical value, however, inherently contain certain errors necessarily resulting from the standard deviation found in their respective testing measurements. Furthermore, when numerical ranges of varying scope are set forth herein, it is contemplated that any combination of these values inclusive of the recited values may be used.

The invention described and claimed herein is not to be limited in scope by the specific embodiments herein disclosed, since these embodiments are intended as illustrations of several aspects of the invention. Any equivalent embodiments are intended to be within the scope of this invention. For example, the compositions of the invention may also be used in golf equipment such as putter inserts, golf club heads and portions thereof, golf shoe portions, and golf bag portions. Indeed, various modifications of the invention in addition to those shown and described herein will become apparent to those skilled in the art from the foregoing description. Such modifications are also intended to fall within the scope of the appended claims. All patents and patent applications cited in the foregoing text are expressly incorporated herein by reference in their entirety.

What is claimed is:

1. A golf ball comprising a core and a cover, wherein the cover comprises a single layer formed from the reaction product of:
  - a conjugated diene comprising a plurality of terminal ends comprising amino groups;
  - an isocyanate-containing component; and
  - a curative blend comprising:
    - an amine-terminated curing agent;
    - a hydroxy-terminated curing agent, wherein at least one of the amine-terminated curing agent and hydroxy-terminated curing agent comprises at least three functional groups; and
    - an organic peroxide;
 wherein the cover has a first hardness at an interior location on the layer at least about 10 percent less than a second hardness at an exterior location on the layer.
2. The golf ball of claim 1, wherein the conjugated diene comprises a polybutadiene.
3. The golf ball of claim 2, wherein the plurality of terminal ends comprise primary amino groups, secondary amino groups, or a combination thereof.
4. The golf ball of claim 1, wherein the first hardness is at least about 12 percent less than the second hardness.

5. The golf ball of claim 1, wherein the first hardness is about 20 percent to about 35 percent less than the second hardness.

6. The golf ball of claim 1, wherein the curative blend further comprises a photoinitiator. 5

7. The golf ball of claim 1, wherein the amine-terminated curing agent is selected from the group consisting of dipropylene triamine, diethylene triamine, propylene oxide based triamine, and combinations thereof.

\* \* \* \* \*

10